



US010838317B2

(12) **United States Patent**  
**Sugahara et al.**

(10) **Patent No.:** **US 10,838,317 B2**  
(45) **Date of Patent:** **Nov. 17, 2020**

(54) **MAGNETIC CARRIER, TWO-COMPONENT DEVELOPER, REPLENISHING DEVELOPER, AND IMAGE FORMING METHOD**

(71) Applicant: **CANON KABUSHIKI KAISHA**,  
Tokyo (JP)

(72) Inventors: **Nobuyoshi Sugahara**, Tokyo (JP);  
**Ryuichiro Matsuo**, Moriya (JP);  
**Hironori Minagawa**, Moriya (JP);  
**Wakashi Iida**, Toride (JP)

(73) Assignee: **CANON KABUSHIKI KAISHA**,  
Tokyo (JP)

(\*) Notice: Subject to any disclaimer, the term of this patent is extended or adjusted under 35 U.S.C. 154(b) by 0 days.

(21) Appl. No.: **16/526,501**

(22) Filed: **Jul. 30, 2019**

(65) **Prior Publication Data**

US 2020/0050123 A1 Feb. 13, 2020

(30) **Foreign Application Priority Data**

Aug. 8, 2018 (JP) ..... 2018-149544

(51) **Int. Cl.**

**G03G 9/00** (2006.01)  
**G03G 9/107** (2006.01)  
**G03G 9/113** (2006.01)  
**G03G 9/083** (2006.01)  
**G03G 9/09** (2006.01)  
**G03G 9/087** (2006.01)

(52) **U.S. Cl.**

CPC ..... **G03G 9/107** (2013.01); **G03G 9/083** (2013.01); **G03G 9/08742** (2013.01); **G03G 9/09** (2013.01); **G03G 9/1075** (2013.01);  
**G03G 9/1131** (2013.01); **G03G 9/1133** (2013.01); **G03G 9/1136** (2013.01)

(58) **Field of Classification Search**

CPC ..... G03G 9/1075; G03G 9/1133  
USPC ..... 430/111.35  
See application file for complete search history.

(56) **References Cited**

U.S. PATENT DOCUMENTS

5,202,210 A 4/1993 Matsuoka et al.  
5,437,949 A 8/1995 Kanbayashi et al.  
(Continued)

FOREIGN PATENT DOCUMENTS

JP H04-188159 A 7/1992  
JP H05-216282 A 8/1993  
(Continued)

OTHER PUBLICATIONS

U.S. Appl. No. 16/531,306, Ryuichiro Matsuo, filed Aug. 5, 2019.  
(Continued)

*Primary Examiner* — Mark A Chapman

(74) *Attorney, Agent, or Firm* — Venable LLP

(57) **ABSTRACT**

A magnetic carrier including a magnetic carrier particle having a magnetic carrier core and a resin coating layer formed on a surface of the magnetic carrier core, wherein the resin coating layer includes a resin component including a resin A and a resin B, the resin A is a copolymer of monomers including (a) a (meth)acrylic acid ester monomer having an alicyclic hydrocarbon group and (b) a specific macromonomer, the resin B is a copolymer of monomers including (c) a styrene-based monomer and (d) a specific (meth)acrylic acid ester monomer, and based on the resin components of the resin coating layer, the amount of the resin A is from 20% by mass to 99% by mass, and the amount of the resin B is from 1% by mass to 80% by mass.

**13 Claims, 4 Drawing Sheets**



(56)

## References Cited

|                       |         |                   |                 |               |                  |
|-----------------------|---------|-------------------|-----------------|---------------|------------------|
| U.S. PATENT DOCUMENTS |         |                   |                 |               |                  |
| 5,607,806 A           | 3/1997  | Kanbayashi et al. | 9,500,975 B2    | 11/2016       | Sugahara et al.  |
| 5,635,326 A           | 6/1997  | Kanbayashi et al. | 9,599,920 B2    | 3/2017        | Sugahara et al.  |
| 5,670,288 A           | 9/1997  | Okado et al.      | 9,606,466 B2    | 3/2017        | Takahashi et al. |
| 5,700,617 A           | 12/1997 | Takiguchi et al.  | 9,665,021 B2    | 5/2017        | Ohtsu et al.     |
| 5,747,209 A           | 5/1998  | Takiguchi et al.  | 9,665,023 B2    | 5/2017        | Kamae et al.     |
| 5,851,714 A           | 12/1998 | Taya et al.       | 9,671,707 B2    | 6/2017        | Minagawa et al.  |
| 5,912,099 A           | 6/1999  | Kanbayashi et al. | 9,703,216 B2    | 7/2017        | Tsuchida et al.  |
| 5,922,500 A           | 7/1999  | Iida et al.       | 9,778,598 B2    | 10/2017       | Onozaki et al.   |
| 5,994,018 A           | 11/1999 | Iida et al.       | 9,785,070 B2    | 10/2017       | Sugahara et al.  |
| 6,013,402 A           | 1/2000  | Kanbayashi et al. | 9,915,885 B2    | 3/2018        | Katsumata et al. |
| 6,022,659 A           | 2/2000  | Kanbayashi et al. | 9,958,809 B2    | 5/2018        | Sugahara et al.  |
| 6,077,635 A           | 6/2000  | Okado et al.      | 9,969,834 B2    | 5/2018        | Ohtsu et al.     |
| 6,326,114 B1          | 12/2001 | Itakura et al.    | 10,007,206 B2   | 6/2018        | Sugahara et al.  |
| 6,528,222 B2          | 3/2003  | Kohtaki et al.    | 10,012,918 B2   | 7/2018        | Ishigami et al.  |
| 6,586,147 B2          | 7/2003  | Iida et al.       | 10,012,921 B2   | 7/2018        | Kamae et al.     |
| 6,664,016 B2          | 12/2003 | Kanbayashi et al. | 10,133,201 B2   | 11/2018       | Kamae et al.     |
| 6,751,424 B2          | 6/2004  | Komatsu et al.    | 10,216,108 B2   | 2/2019        | Iwasaki et al.   |
| 6,808,852 B2          | 10/2004 | Hotta et al.      | 10,234,777 B2   | 3/2019        | Ohtsu et al.     |
| 6,929,894 B2          | 8/2005  | Sugahara et al.   | 10,409,188 B2   | 9/2019        | Sugahara et al.  |
| 7,022,449 B2          | 4/2006  | Sugahara et al.   | 10,423,090 B2   | 9/2019        | Ohtsu et al.     |
| 7,115,349 B2          | 10/2006 | Iida et al.       | 10,451,985 B2   | 10/2019       | Takahashi et al. |
| 7,138,213 B2          | 11/2006 | Itakura et al.    | 2014/0137428 A1 | 5/2014        | Takenaka et al.  |
| 7,144,668 B2          | 12/2006 | Baba et al.       | 2018/0275540 A1 | 9/2018        | Matsuo et al.    |
| 7,147,980 B2          | 12/2006 | Itakura et al.    | 2019/0155182 A1 | 5/2019        | Watanabe et al.  |
| 7,279,262 B2          | 10/2007 | Fujikawa et al.   |                 |               |                  |
| 7,288,348 B2          | 10/2007 | Hayami et al.     | JP              | H08-179569 A  | 7/1996           |
| 7,297,455 B2          | 11/2007 | Fujikawa et al.   | JP              | H10-010789 A  | 1/1998           |
| 7,396,626 B2          | 7/2008  | Fujikawa et al.   | JP              | 2014-077902 A | 5/2014           |
| 7,396,629 B2          | 7/2008  | Baba et al.       | JP              | 2016-048369 A | 4/2016           |
| 7,442,478 B2          | 10/2008 | Itakura et al.    | JP              | 2016-170216 A | 9/2016           |
| 7,455,947 B2          | 11/2008 | Ida et al.        | JP              | 2017-044792 A | 3/2017           |
| 7,536,132 B2          | 5/2009  | Minagawa          |                 |               |                  |
| 7,544,457 B2          | 7/2009  | Hashimoto et al.  |                 |               |                  |
| 7,816,063 B2          | 10/2010 | Hashimoto et al.  |                 |               |                  |
| 9,046,800 B2          | 6/2015  | Hotta et al.      |                 |               |                  |
| 9,075,328 B2          | 7/2015  | Minagawa et al.   |                 |               |                  |
| 9,158,217 B2          | 10/2015 | Takahashi et al.  |                 |               |                  |
| 9,372,420 B2          | 6/2016  | Mizo et al.       |                 |               |                  |
| 9,454,094 B2          | 9/2016  | Tsujimoto et al.  |                 |               |                  |

## FOREIGN PATENT DOCUMENTS

|    |               |        |
|----|---------------|--------|
| JP | H08-179569 A  | 7/1996 |
| JP | H10-010789 A  | 1/1998 |
| JP | 2014-077902 A | 5/2014 |
| JP | 2016-048369 A | 4/2016 |
| JP | 2016-170216 A | 9/2016 |
| JP | 2017-044792 A | 3/2017 |

## OTHER PUBLICATIONS

- U.S. Appl. No. 16/539,245, Ryuji Murayama, filed Aug. 13, 2019.  
 U.S. Appl. No. 16/550,418, Daisuke Tsujimoto, filed Aug. 26, 2019.  
 U.S. Appl. No. 16/550,452, Takeshi Ohtsu, filed Aug. 26, 2019.  
 U.S. Appl. No. 16/561,168, Toru Takahashi, filed Sep. 5, 2019.  
 U.S. Appl. No. 16/571,427, Nobuyoshi Sugahara, filed Sep. 16, 2019.



**Fig. 1**



Fig. 2



**Fig. 3**



Fig. 4

## 1

**MAGNETIC CARRIER, TWO-COMPONENT  
DEVELOPER, REPLENISHING DEVELOPER,  
AND IMAGE FORMING METHOD**

## BACKGROUND OF THE INVENTION

## Field of the Invention

The present invention relates to a magnetic carrier, a two-component developer, and a replenishing developer to be used in an image forming method for visualizing an electrostatic charge image by using electrophotography, and to an image forming method using the same.

## Description of the Related Art

Conventionally, a method of forming an electrostatic latent image by using various means on an electrostatic latent image bearing member, attaching a toner to the electrostatic latent image, and developing the electrostatic latent image have been generally used as an electrophotographic image forming method. A two-component development system in which carrier particles called magnetic carrier are mixed with a toner and triboelectrically charged to apply a suitable amount of positive or negative charge to the toner, and development is performed using the charge as a driving force has been widely used in such development.

The merit of the two-component development method is that functions such as stirring, transport, and charging of the developer can be imparted to the magnetic carrier, so that functions can be clearly divided between the magnetic carrier and the toner, thereby ensuring satisfactory controllability of the developer performance.

Meanwhile, in recent years, technological advances in the field of electrophotography created an ever-growing demand for a higher speed and longer life of devices and also for higher definition and stable image quality. In order to meet such demands, higher performance of magnetic carriers is needed.

Among them, Japanese Patent Application Publication No. 2014-077902, Japanese Patent Application Publication No. 2016-048369, and Japanese Patent Application Publication No. 2017-044792 disclose coating resins which improve the adhesion with the carrier core, reduce the concentration fluctuation even in long-term use, and stabilize the charge quantity even when allowed to stand for a long time. These carriers are characterized in that a copolymer of a specific (meth)acrylic acid monomer and a specific macromonomer is used as a coating resin.

Further, Japanese Patent Application Publication No. 2016-170216 and Japanese Patent Application Publication No. H04-188159 propose examples in which a (meth)acrylic acid monomer is used as a coating resin, and Japanese Patent Application Publication No. H08-179569 proposes an example in which a macromonomer is used.

Further, Japanese Patent Application Publication No. H05-216282 and Japanese Patent Application Publication No. H10-010789 propose using coating resins having improved charging stability and environmental characteristics.

## SUMMARY OF THE INVENTION

With the magnetic carriers of the above-mentioned patent documents, the service life has been extended and the ability to follow environmental changes has been improved.

## 2

However, in the market, particularly in the field of on-demand printers, there is an increasing demand for stably obtaining high-quality images, such that have color tone stability of images during long-term use, in-plane uniformity of halftone and the like. There is an urgent need to develop a magnetic carrier, a two-component developer, and an image forming method using the same, which meet such a demand.

One aspect of the present invention is directed to providing a magnetic carrier which solves the above problems. Specifically, the present invention is to provide a magnetic carrier capable of improving the color tone stability of images and in-plane uniformity of halftone and producing images stable against environmental fluctuations.

By using a magnetic carrier as shown below, it is possible to reduce the environmental difference in charge-providing performance even when the mode is switched from long-term use at low print density to use at high print density. In addition, color tone variation of the image is suppressed, the in-plane uniformity of halftone is improved, and a high-quality image can be obtained.

That is, one aspect of the present invention provides a magnetic carrier comprising a magnetic carrier particle, wherein

the magnetic carrier particle contains a magnetic carrier core and a resin coating layer formed on a surface of the magnetic carrier core,

the resin coating layer includes a resin component including a resin A and a resin B,

the resin A is a copolymer of monomers including

(a) a (meth)acrylic acid ester monomer having an alicyclic hydrocarbon group, and

(b) a macromonomer containing a polymer portion and a reactive portion bound to the polymer portion, wherein

the polymer portion has a polymer of at least one monomer selected from the group consisting of methyl

acrylate, methyl methacrylate, butyl acrylate, butyl methacrylate, 2-ethylhexyl acrylate and 2-ethylhexyl methacrylate, and

the reactive portion has a reactive C—C double bond, the resin B is a copolymer of monomers including

(c) a styrene-based monomer, and

(d) a (meth)acrylic acid ester monomer having a hydroxy group and represented by a following formula (1), and

based on the resin components of the resin coating layer, the amount of the resin A is from 20% by mass to 99% by mass, and the amount of the resin B is from 1% by mass to 80% by mass.



(In the formula (1), R represents H or  $\text{CH}_3$ , and n represents an integer of from 1 to 8).

Another aspect of the present invention provides a two-component developer including

a toner comprising a toner particle including a binder resin, and

a magnetic carrier,

wherein

the magnetic carrier is the abovementioned magnetic carrier.

Another aspect of the present invention provides a replenishing developer for use in an image forming method which comprises:

a charging step of charging an electrostatic latent image bearing member;

an electrostatic latent image forming step of forming an electrostatic latent image on a surface of the electrostatic latent image bearing member;

a developing step of developing the electrostatic latent image by using a two-component developer in a developing device to form a toner image;

a transfer step of transferring the toner image to a transfer material with or without an intermediate transfer member; and

a fixing step of fixing the transferred toner image to the transfer material, and

in which the replenishing developer is replenished to the developing device in accordance with a reduction in toner concentration in the two-component developer in the developing device, wherein

the replenishing developer includes a magnetic carrier and a toner having a toner particle including a binder resin,

the replenishing developer includes from 2 parts by mass to 50 parts by mass of the toner with respect to 1 part by mass of the magnetic carrier, and

the magnetic carrier is the abovementioned magnetic carrier.

The present invention also relates to an image forming method comprising:

a charging step of charging an electrostatic latent image bearing member;

an electrostatic latent image forming step of forming an electrostatic latent image on a surface of the electrostatic latent image bearing member;

a developing step of developing the electrostatic latent image by using a two-component developer in a developing device to form a toner image;

a transfer step of transferring the toner image to a transfer material with or without an intermediate transfer member; and

a fixing step of fixing the transferred toner image to the transfer material, wherein

the two-component developer is the abovementioned two-component developer.

Still another aspect of the present invention provides an image forming method which comprises:

a charging step of charging an electrostatic latent image bearing member;

an electrostatic latent image forming step of forming an electrostatic latent image on a surface of the electrostatic latent image bearing member;

a developing step of developing the electrostatic latent image by using a two-component developer in a developing device to form a toner image;

a transfer step of transferring the toner image to a transfer material with or without an intermediate transfer member; and

a fixing step of fixing the transferred toner image to the transfer material, and

in which a replenishing developer is replenished to the developing device in accordance with a reduction in toner concentration in the two-component developer in the developing device, wherein

the replenishing developer includes a magnetic carrier and a toner having a toner particle including a binder resin,

the replenishing developer includes from 2 parts by mass to 50 parts by mass of the toner with respect to 1 part by mass of the magnetic carrier, and

the magnetic carrier is the abovementioned magnetic carrier.

With the present invention, it is possible to obtain a magnetic carrier capable of improving the color tone stability of images and the in-plane uniformity of halftone and producing images stable against environmental fluctuations.

Further features of the present invention will become apparent from the following description of exemplary embodiments with reference to the attached drawings.

#### BRIEF DESCRIPTION OF THE DRAWINGS

FIG. 1 is a schematic view of an image forming apparatus;

FIG. 2 is a schematic view of an image forming apparatus;

FIG. 3 is a schematic view of a method for specifying the amount of coating resin in a GPC molecular weight distribution curve; and

FIG. 4 is a schematic view of a method for specifying the amount of coating resin in a GPC molecular weight distribution curve.

#### DESCRIPTION OF THE EMBODIMENTS

In the present invention, the expressions "from XX to YY" or "XX to YY" representing a numerical range mean a numerical range including the lower limit and the upper limit which are endpoints, unless otherwise noted.

In the present invention, a (meth)acrylic acid ester means an acrylic acid ester and/or a methacrylic acid ester.

The magnetic carrier of the present invention has a magnetic carrier particle having a magnetic carrier core and a resin coating layer formed on a surface of the magnetic carrier core, wherein

the resin coating layer includes a resin component including a resin A and a resin B,

the resin A is a copolymer of monomers including

(a) a (meth)acrylic acid ester monomer having an alicyclic hydrocarbon group, and

(b) a macromonomer containing a polymer portion and a reactive portion bound to the polymer portion, wherein

the polymer portion has a polymer of at least one monomer selected from the group consisting of methyl acrylate, methyl methacrylate, butyl acrylate, butyl methacrylate, 2-ethylhexyl acrylate and 2-ethylhexyl methacrylate, and

the reactive portion has a reactive C—C double bond, the resin B is a copolymer of monomers including

(c) a styrene-based monomer, and

(d) a (meth)acrylic acid ester monomer having a hydroxy group and represented by the following formula (1), and

based on the resin components of the resin coating layer, the amount of the resin A is from 20% by mass to 99% by mass, and the amount of the resin B is from 1% by mass to 80% by mass.



(In the formula (1), R represents H or  $\text{CH}_3$ , and n represents an integer of from 1 to 8 (preferably from 1 to 6)).

Usually, when the mode of use is switched from long-term use at low print density to use at high print density, a charge difference occurs between the toner in the developer and the newly supplied toner. As a result, color tone variation in the image plane and density unevenness in halftone occur. Although there is a method of rapidly providing a charge to a toner by designing a coating resin with high charge-providing performance in order to minimize the charge difference of the toner, there is a concern that the environmental difference in charge-providing performance increases.

The inventors of the present invention have conducted a comprehensive study for the purpose of achieving both the extension of the developer life and the suppression of color tone variation in the image plane in long-term use and density unevenness in halftone. As a result, it has been found that the abovementioned specific magnetic carrier is important.

It has been found that the configuration of the present invention makes it possible to accelerate the charge buildup regardless of the environment, and to suppress the charge decrease in a high-humidity environment and the excessive charge in a low-humidity environment. It is believed that the interaction between the macromonomer component of the resin A and the hydroxy group of the resin B is effective in increasing the chargeability particularly in a high-humidity environment. Further, it is considered that the interaction between the styrene component and the alicyclic hydrocarbon group has an effect of suppressing excessive charging in a low-humidity environment.

Furthermore, it is believed that the macromonomer component and the hydroxy group are more effective as a result of being incorporated into different molecular structures, as in the configuration of the present invention, rather than in the same molecule. Likewise, it is believed that the alicyclic hydrocarbon group and the styrene component are more effective as a result of being incorporated into different molecular structures.

The amount of the resin A is from 20% by mass to 99% by mass, and the amount of the resin B is from 1% by mass to 80% by mass based on the resin component of the resin coating layer. In these ranges, the environmental difference in charging performance can be reduced. The amount of the resin A is preferably from 25% by mass to 90% by mass, and the amount of the resin B is preferably from 10% by mass to 75% by mass.

In addition, it is preferable that the sum total of the amount of the resin A and the amount of the resin B is from 80% by mass to 100% by mass, and more preferably 90% by mass to 100% by mass based on the resin component.

Examples of the resin component of the resin coating layer other than the resin A and the resin B include vinyl resins and polyester resins, but preferably a resin which hardly affects the interaction of the resin A and the resin B, and a resin which does not have an acid value or a hydroxyl value. Among them, more preferable resins include poly(meth)acrylic acid esters such as poly(methyl methacrylate) and poly(methyl acrylate).

The hydroxyl value of the resin component contained in the resin coating layer is preferably from 0.5 mg KOH/g to 10.0 mg KOH/g, and more preferably from 1.0 mg KOH/g to 8.5 mg KOH/g. By setting the hydroxyl value within the above range, an environmental difference in charging performance can be further reduced.

Further, based on the mass of the monomers forming the resin component included in the resin coating layer, the proportion of the sum total of the (meth)acrylic acid ester

monomer having an alicyclic hydrocarbon group and the styrene-based monomer is preferably from 50.0% by mass to 95.0% by mass, and more preferably from 60.0% by mass to 90.0% by mass. When the amount is 50.0% by mass or more, color tone stability is increased.

On the other hand, when the amount is 95.0% by mass or less, in-plane uniformity of halftone is improved.

Further, based on the mass of the monomers forming the resin component included in the resin coating layer, the proportion of the (meth)acrylic acid ester monomer having an alicyclic hydrocarbon group is preferably from 5.0% by mass to 80.0% by mass, and more preferably from 10.0% by mass to 60.0% by mass. Within these ranges, a change in color tone in a high-temperature and high-humidity environment is reduced.

Meanwhile, based on the mass of the monomers forming the resin component included in the resin coating layer, the proportion of the styrene-based monomer is preferably from 0.8% by mass to 70.0% by mass, and more preferably from 7.0% by mass to 60.0% by mass. Within these ranges, a color tone variation and in-plane uniformity of halftone are likely to be increased.

#### Resin A

The resin A used for the resin coating layer is a vinyl-based resin which is a copolymer of monomers including a vinyl-based monomer having a cyclic hydrocarbon group in a molecular structure and another vinyl-based monomer. Among them, it is necessary that the resin A is a copolymer of a (meth)acrylic ester having an alicyclic hydrocarbon group and a monomer including a specific macromonomer. A monomer other than the (meth)acrylic acid ester having an alicyclic hydrocarbon group and the specific macromonomer may also be used to the extent that the effects of the present invention are not impaired.

In the resin A, the polymer portion of the monomer including a (meth)acrylic acid ester having an alicyclic hydrocarbon group makes the coated surface of the resin layer coated on the surface of the magnetic carrier core smooth. As a result, this portion acts to suppress the adhesion of a toner-derived component to the magnetic carrier and to suppress the decrease of charging performance. In addition, the macromonomer portion improves the adhesion with the magnetic carrier core, thereby improving the image density stability. Furthermore, charge leakage in the coated thin layer portion can be reduced in a high-humidity environment over a long period of time, and the density after storage and fine line reproducibility can be stabilized.

Examples of the (meth)acrylic acid ester (monomer) having an alicyclic hydrocarbon group include cyclobutyl acrylate, cyclopentyl acrylate, cyclohexyl acrylate, cycloheptyl acrylate, dicyclopentenyl acrylate, dicyclopentenyl acrylate, cyclobutyl methacrylate, cyclopentyl methacrylate, cyclohexyl methacrylate, cycloheptyl methacrylate, dicyclopentenyl methacrylate, dicyclopentenyl methacrylate and the like. The alicyclic hydrocarbon group is preferably a cycloalkyl group, and the carbon number is preferably from 3 to 10, and more preferably from 4 to 8. One or two or more of these may be selected and used.

The macromonomer contains a polymer portion and a reactive portion bound to the polymer portion. The polymer portion has a polymer of at least one monomer selected from the group consisting of methyl acrylate, methyl methacrylate, butyl acrylate, butyl methacrylate, 2-ethylhexyl acrylate, and 2-ethylhexyl methacrylate. The reactive portion has a reactive C=C double bond. The macromonomer can be exemplified by a polymer of at least one monomer selected from the group consisting of methyl acrylate, methyl meth-

acrylate, butyl acrylate, butyl methacrylate, 2-ethylhexyl acrylate, and 2-ethylhexyl methacrylate. Example of the reactive portion having reactive C—C double bond includes vinyl group, acryloyl group and methacryloyl group.

The proportion of the macromonomer is preferably from 15.0% by mass to 40.0% by mass, and more preferably from 20.0% by mass to 35.0% by mass based on the mass of the monomers for forming the resin A.

By setting the proportion of the macromonomer within the abovementioned ranges, it is possible to maintain the toughness and abrasive resistance of the resin coating layer and to further decrease the environmental difference in charging performance in combination with the resin B.

Further, the hydroxyl value of the resin A is preferably from 0 mg KOH/g to 1.0 mg KOH/g, and more preferably from 0 mg KOH/g to 0.8 mg KOH/g.

By setting the hydroxyl value within the abovementioned ranges, it is possible to further decrease the environmental difference in charging performance in combination with the resin B.

From the viewpoint of stability of the coating, the weight average molecular weight (Mw) of the resin A is preferably from 20,000 to 75,000, and more preferably from 25,000 to 70,000.

In the resin A, a (meth)acrylic monomer other than the (meth)acrylic acid ester having an alicyclic hydrocarbon group and the macromonomer may be used as a monomer.

Examples of the other (meth)acrylic monomer include methyl acrylate, methyl methacrylate, ethyl acrylate, ethyl methacrylate, butyl acrylate (n-butyl, sec-butyl, iso-butyl or tert-butyl; the same applies hereinafter), butyl methacrylate, 2-ethylhexyl acrylate, 2-ethylhexyl methacrylate, acrylic acid, methacrylic acid and the like.

The proportion of the other (meth)acrylic monomer is preferably from 0% by mass to 10% by mass based on the mass of the monomers for forming the resin A.

The weight average molecular weight Mw of the macromonomer determined by gel permeation chromatography is preferably from 1000 to 9500. When the weight average molecular weight of the macromonomer is from 1000 to 9500, adhesion between the magnetic carrier core particles and the resin coating layer and charging stability are improved, so that color tone variation and in-plane uniformity of halftone are likely to be improved.

#### Resin B

The resin B is a copolymer of a monomer including a styrene-based monomer and a (meth)acrylic acid ester monomer having a hydroxy group and represented by the formula (1). By including the styrene-based monomer in the copolymer, it is possible to increase the glass transition point even with the same molecular weight as compared with a resin containing no styrene-based monomer, and the toughness of the resin coating layer can be maintained even with a low molecular weight. To the extent that the effects of the present invention are not impaired, monomers other than the styrene-based monomer and the (meth)acrylic acid ester monomer having a hydroxy group and represented by the formula (1) may be used.

Further, by including the (meth)acrylic acid ester monomer having a hydroxy group and represented by the formula (1), the affinity with the macromonomer of the resin A having a similar structure is enhanced. Therefore, the toughness and abrasion resistance of the resin coating layer are improved, and color tone variation and in-plane uniformity of halftone are likely to be improved.

The styrene-based monomer is not particularly limited, and suitable examples thereof are presented hereinbelow.

Styrene; styrene derivatives such as  $\alpha$ -methylstyrene,  $\beta$ -methylstyrene,  $\alpha$ -methylstyrene, m-methylstyrene, p-methylstyrene, 2,4-dimethylstyrene, p-n-butylstyrene, p-tert-butylstyrene, p-n-hexylstyrene, p-n-octylstyrene, p-n-nonylstyrene, p-n-decylstyrene, p-n-dodecylstyrene, p-methoxystyrene, p-phenylstyrene and the like.

The resin to be used as the resin B is not particularly limited. Examples of suitable resins include styrene copolymers such as a styrene-2-hydroxyethyl acrylate copolymer, 10 a styrene-2-hydroxyethyl methacrylate copolymer and the like. These may be used singly or in combination of two or more types thereof.

The peak molecular weight in the molecular weight distribution of the resin B determined by gel permeation 15 chromatography (GPC) is preferably from 3000 to 20,000, more preferably from 5000 to 20,000, and still more preferably from 5500 to 19,000. When the peak molecular weight of the resin B is 3000 or more, the effect of improving the toughness and abrasion resistance of the resin 20 coating layer and reducing the environmental difference in charging performance is enhanced. Meanwhile, when the peak molecular weight is 20,000 or less, the color tone stability and in-plane uniformity of the halftone are further improved. The peak molecular weight is taken as the 25 molecular weight at the highest peak.

The proportion of the (meth)acrylic acid ester monomer having a hydroxy group and represented by the formula (1) is preferably from 0.1% by mass to 3.0% by mass, and more 30 preferably from 0.5% by mass to 2.5% by mass based on the mass of the monomers forming the resin component contained in the resin coating layer.

Further, the hydroxyl value of the resin B is preferably from 0.2 mg KOH/g to 30.0 mg KOH/g or less, more 35 preferably from 5.0 mg KOH/g to 30.0 mg KOH/g, and still more preferably from 5.0 mg KOH/g to 15.0 mg KOH/g.

By setting the proportion of the (meth)acrylic acid ester monomer having a hydroxy group in the above ranges and the hydroxyl value of the resin B, an environmental difference in charging performance can be further reduced.

40 The amount of the resin coating layer is preferably from 1.0 part by mass to 3.0 parts by mass with respect to 100 parts by mass of the magnetic carrier core. When the amount is 1.0 part by mass or more, the toughness and abrasion resistance of the resin are increased and a change in the 45 image density is suppressed. Meanwhile, when the amount is 3.0 parts by mass or less, the charge relaxation property is further enhanced, and density unevenness in the image plane and the decrease in fine line reproducibility are further suppressed.

50 Next, the magnetic carrier core used in the present invention will be described.

A well-known magnetic carrier core can be used as the 55 magnetic carrier core used for the magnetic carrier of this invention. It is more preferable to use a magnetic body-dispersed resin particle in which a magnetic body is dispersed in a resin component, or a porous magnetic core particle including a resin in a void portion.

These can reduce the true density of the magnetic carrier, and hence can reduce the load on the toner. As a result, even 60 in long-term use, the deterioration of image quality is small and it is possible to reduce the replacement frequency of the developer composed of the toner and the carrier. However, these magnetic carrier cores are not limiting, and the effects of the present invention can be sufficiently exhibited even if 65 a commercially available magnetic carrier core is used.

Examples of the magnetic body component to be used for the magnetic body-dispersed resin particle include various

magnetic iron compound particle powders such as magnetite particle powder, maghemite particle powder, and magnetic iron oxide particle powder obtained by including at least one selected from silicon oxide, silicon hydroxide, aluminum oxide, and aluminum hydroxide therein; magnetoplumbite type ferrite particle powder including barium, strontium or barium-strontium; spinel type ferrite particle powder including at least one selected from manganese, nickel, zinc, lithium and magnesium; and the like.

Among these, magnetic iron oxide particle powders are preferably used.

In addition to the magnetic body component, nonmagnetic iron oxide particle powder such as hematite particle powder, nonmagnetic hydrous ferric oxide particle powder such as goethite particle powder, and nonmagnetic inorganic compound particle powder such as titanium oxide particle powder, silica particle powder, talc particle powder, alumina particle powder, barium sulfate particle powder, barium carbonate particle powder, cadmium yellow particle powder, calcium carbonate particle powder, zinc oxide particle powder, and the like may be used in combination with the magnetic iron compound particle powder.

When the magnetic iron compound particle powder and the nonmagnetic inorganic compound particle powder are used in a mixture, it is preferable that the magnetic iron compound particle powder be included at a mixing ratio of at least 30% by mass.

It is preferable that the magnetic iron compound particle powder be entirely or partially treated with a lipophilic agent.

In this case, an organic compound having one or two or more functional groups such as an epoxy group, an amino group, a mercapto group, an organic acid group, an ester group, a ketone group, a halogenated alkyl group and an aldehyde group, or a mixture of such organic compounds can be used for the lipophilic treatment.

The organic compound having a functional group is preferably a coupling agent, more preferably a silane coupling agent, a titanium coupling agent and an aluminum coupling agent, and a silane coupling agent is particularly preferable.

A thermosetting resin is preferable as a binder resin constituting the magnetic body-dispersed resin particle. For example, a phenol resin, an epoxy resin, an unsaturated polyester resin and the like can be used, but from the viewpoint of inexpensiveness and easiness of the production method, it is preferable that a phenol resin be included. For example, a phenol-formaldehyde resin can be mentioned.

The content ratio of the binder resin and the magnetic iron compound particle powder (or the mixture of the magnetic iron compound particle powder and the nonmagnetic inorganic compound particle powder) constituting the composite particle in the present invention is preferably from 1% by mass to 20% by mass of the binder resin and from 80% by mass to 99% by mass of the magnetic iron compound particle powder (or the mixture).

Next, a method for producing the magnetic body-dispersed resin particle will be described.

A phenol and an aldehyde are stirred in an aqueous medium in the presence of magnetic and nonmagnetic inorganic compound particle powders and a basic catalyst, for example, as indicated in Examples described hereinbelow. Then, the phenol and the aldehyde are reacted and cured to generate a composite particle including an inorganic compound particle such as magnetic iron particle powder and a phenol resin.

Moreover, the magnetic body-dispersed resin particle can be also manufactured by the so-called knead-pulverizing method by which a binder resin including inorganic compound particles such as magnetic iron oxide particle powder is pulverized. The former method is preferred because the particle diameter of the magnetic carrier can be easily controlled and a sharp particle diameter distribution can be obtained.

Next, a porous magnetic core particle will be described.

As a material of the porous magnetic core particle, magnetite or ferrite is preferable. Furthermore, ferrite is more preferable as the material of the porous magnetic core particle because the porous structure of the porous magnetic core particle can be controlled and the resistance can be adjusted.

Ferrite is a sintered body represented by a following general formula.



(wherein, M1 is a monovalent metal, M2 is a divalent metal, and x and y each satisfy  $0 \leq (x, y) \leq 0.8$  where  $x+y+z=1.0$ , and z is  $0.2 < z < 1.0$ )

In the formula, at least one metal atom selected from the group consisting of Li, Fe, Mn, Mg, Sr, Cu, Zn, Ca is preferably used as M1 and M2. In addition, Ni, Co, Ba, Y, V, Bi, In, Ta, Zr, B, Mo, Na, Sn, Ti, Cr, Al, Si, rare earths and the like can be used.

In the magnetic carrier, it is preferable to maintain the appropriate amount of magnetization and to control the unevenness state of the surface of the porous magnetic core particle in order to bring the fine pore diameter into a desired range. In addition, it is preferable that the rate of the ferritization reaction could be easily controlled, and the specific resistance and magnetic force of the porous magnetic core could be suitably controlled. From the above viewpoints, a Mn-based ferrite, a Mn—Mg-based ferrite, a Mn—Mg—Sr-based ferrite, and a Li—Mn-based ferrite including a Mn element are more preferable. A manufacturing process implemented in the case of using a porous ferrite particle as a magnetic carrier core is explained hereinbelow in detail.

#### Step 1 (Weighing and Mixing Step)

The raw materials of the above ferrite are weighed and mixed. The ferrite raw materials can be exemplified by metal particle of the abovementioned metal elements, or oxides, hydroxides, oxalates, carbonates and the like thereof.

Examples of an apparatus for mixing are presented hereinbelow. A ball mill, a planetary mill, a Giotto mill, and a vibration mill. In particular, a ball mill is preferable from the viewpoint of mixability.

Specifically, the weighed ferrite raw materials and balls are placed in a ball mill, and pulverized and mixed, preferably for 0.1 h to 20.0 h.

#### Step 2 (Pre-baking Step)

The pulverized and mixed ferrite raw materials are pre-baked in the air or in a nitrogen atmosphere, preferably at a baking temperature of from 700° C. to 1200° C., preferably for 0.5 h to 5.0 h, to form a ferrite. For example, the following furnace is used for firing. A burner type baking furnace, a rotary type baking furnace, an electric furnace and the like.

#### Step 3 (Pulverization Step)

The pre-baked ferrite produced in step 2 is pulverized in a pulverizer.

The pulverizer is not particularly limited as long as a desired particle diameter can be obtained. For example, the

## 11

following can be mentioned. A crusher, a hammer mill, a ball mill, a bead mill, a planetary mill, a Giotto mill and the like.

In order to obtain the desired particle diameter of the pulverized ferrite product, it is preferable to control the material of the balls or beads used in a ball mill or bead mill, the particle diameter, and the operation time. Specifically, in order to reduce the particle diameter of the pre-baked ferrite slurry, balls with a high specific gravity may be used or the pulverizing time may be lengthened. Moreover, in order to widen the particle size distribution of the pre-baked ferrite, balls or beads with a high specific gravity may be used or the pulverizing time can be lengthened. Also, by mixing a plurality of pre-baked ferrites different in particle diameter, it is possible to obtain a pre-baked ferrite having a wide distribution.

Further, in the ball mill and bead mill, a wet method is superior to a dry method in that the pulverized product does not fly up in the mill and the pulverizing efficiency is high. Therefore, the wet method is more preferable than the dry method.

## Step 4 (Granulation Step)

Water, a binder and, if necessary, a pore regulator are added to the pulverized product of pre-baked ferrite. The pore regulator can be exemplified by a foaming agent and fine resin particles.

The foaming agent can be exemplified by sodium hydrogencarbonate, potassium hydrogencarbonate, lithium hydrogencarbonate, ammonium hydrogencarbonate, sodium carbonate, potassium carbonate, lithium carbonate, and ammonium carbonate.

The fine resin particles can be exemplified by polyesters, polystyrene, and styrene copolymers such as styrene-vinyl toluene copolymer, styrene-vinyl naphthalene copolymer, styrene-acrylic acid ester copolymer, styrene-methacrylic acid ester copolymer, styrene- $\alpha$ -chloromethacrylic acid, styrene-acrylonitrile copolymer, styrene-vinyl methyl ketone copolymer, styrene-butadiene copolymer, styrene-isoprene copolymer, styrene-acrylonitrile-indene copolymer and the like; polyvinyl chloride, phenol resins, modified phenol resins, maleic resins, acrylic resins, methacrylic resins, polyvinyl acetate, and silicone resins; polyester resins having monomers selected from aliphatic polyhydric alcohols, aliphatic dicarboxylic acids, aromatic dicarboxylic acids, aromatic dialcohols and diphenols as structural units; polyurethane resins, polyamide resins, polyvinyl butyral, terpene resins, coumarone indene resins, petroleum resins, and hybrid resins having a polyester unit and a vinyl polymer unit.

For example, polyvinyl alcohol can be used as the binder.

In step 3, in the case of wet pulverizing, it is preferable to add a binder and, if necessary, a pore regulator by taking into consideration the water contained in the ferrite slurry.

The obtained ferrite slurry is dried and granulated using a spray drying device, preferably in a heating atmosphere at from 100° C. to 200° C. The spray drying device is not particularly limited as long as the desired particle diameter of the porous magnetic core particles can be obtained. For example, a spray dryer can be used.

## Step 5 (Main Baking Step)

Next, the granulated product is baked, preferably at 800° C. to 1400° C., and preferably for 1 h to 24 h.

By raising the baking temperature and prolonging the baking time, baking of the porous magnetic core particles is promoted, and as a result, the pore diameter is decreased and the number of pores is also reduced.

## 12

## Step 6 (Sorting Step)

After pulverizing the baked particles as described above, if necessary, coarse particles or fine particles may be removed by classification or screening with a sieve.

From the viewpoint of suppression of carrier adhesion and attachment to an image, the volume distribution standard 50% particle diameter (D50) of the magnetic core particles is preferably from 18.0  $\mu$ m to 68.0  $\mu$ m.

## Step 7 (Filling Step)

Depending on the pore volume thereinside, the porous magnetic core particle may have a low physical strength, and in order to increase the physical strength as a magnetic carrier, at least a part of the voids of the porous magnetic core particle is preferably filled with a resin. The amount of the resin filled in the porous magnetic core particles is preferably 2% by mass to 15% by mass in the porous magnetic core particles.

Provided that the spread in the resin amount for each magnetic carrier is small, the resin may be filled in only a part of the internal voids, the resin may be filled only in the voids near the surface of the porous magnetic core particle while the voids remain inside, or the internal voids may be completely filled with the resin.

A method for filling the resin in the voids of the porous magnetic core particles is not particularly limited. For example, a method can be used by which a porous magnetic core particle is impregnated with a resin solution by a coating method such as an immersion method, a spray method, a brushing method and a fluidized bed, and the solvent is thereafter evaporated. Further, a method can also be used by which a resin is diluted with a solvent and then added to the voids in the porous magnetic core particle.

The solvent used here may be any one that can dissolve the resin. When the resin is soluble in an organic solvent, examples of the organic solvent include toluene, xylene, cellosolve butyl acetate, methyl ethyl ketone, methyl isobutyl ketone and methanol. In the case of a water-soluble resin or an emulsion-type resin, water may be used as the solvent.

The amount of solid resin fraction in the resin solution is preferably 1% by mass to 50% by mass, and more preferably 1% by mass to 30% by mass. When the amount is 50% by mass or less, the viscosity is not too high, and the resin solution easily penetrates uniformly into the voids of the porous magnetic core particles. Meanwhile, when the amount is 1% by mass or more, the amount of resin is appropriate, and the adhesion of the resin to the porous magnetic core particle is improved.

Either a thermoplastic resin or a thermosetting resin may be used as a resin for filling the voids of the porous magnetic core particles. A resin with high affinity to the porous magnetic core particle is preferable. When a resin having high affinity is used, the surface of the porous magnetic core particle can be covered with the resin simultaneously with the filling of the resin into the voids of the porous magnetic core particle.

Examples of the thermoplastic resin as the resin to be filled are as follows. A novolak resin, a saturated alkyl polyester resin, a polyarylate, a polyamide resin, an acrylic resin and the like.

Examples of the thermosetting resin are as follows. A phenol resin, an epoxy resin, an unsaturated polyester resin, a silicone resin and the like.

Further, the magnetic carrier has a resin coating layer on the surface of the magnetic carrier core.

A method for coating the surface of the magnetic carrier core with a resin is not particularly limited, and examples

thereof include a coating method by an immersion method, a spray method, a brush coating method, a dry method, and a fluidized bed.

Further, conductive particles and particles and materials having charge controllability may be contained in the resin coating layer. Examples of conductive particles include carbon black, magnetite, graphite, zinc oxide and tin oxide.

The amount of conductive particles added is preferably 0.1 parts by mass to 10.0 parts by mass with respect to 100 parts by mass of the coating resin in order to adjust the resistance of the magnetic carrier.

Examples of particles having charge controllability include particles of organic metal complexes, particles of organic metal salts, particles of chelate compounds, particles of monoazo metal complexes, particles of acetylacetone metal complexes, particles of hydroxycarboxylic acid metal complexes, particles of polycarboxylic acid metal complexes, particles of polyol metal complexes, particles of polymethyl methacrylate resin, particles of polystyrene resin, particles of melamine resin, particles of phenol resin, particles of nylon resin, particles of silica, particles of titanium oxide, particles of alumina and the like.

The addition amount of the particles having charge controllability is preferably 0.5 parts by mass to 50.0 parts by mass with respect to 100 parts by mass of the coating resin in order to adjust the triboelectric charge quantity.

Next, the preferred toner configuration is described in detail below.

The toner has a toner particle including a binder resin and, as necessary, a colorant and a release agent. The binder resin may be exemplified by a vinyl resin, a polyester resin, an epoxy resin and the like. Among them, a vinyl resin and a polyester resin are more preferable in terms of charging performance and fixability. A polyester resin is particularly preferred.

Homopolymers or copolymers of vinyl monomers, polyesters, polyurethanes, epoxy resins, polyvinyl butyral, rosins, modified rosins, terpene resins, phenol resins, aliphatic or alicyclic hydrocarbon resins, aromatic petroleum resins, and the like can be used, if necessary, by mixing with the above-mentioned binder resin.

When two or more kinds of resins are mixed and used as a binder resin, in a more preferable embodiment, it is preferable that the resins having different molecular weights be mixed in a suitable proportion.

The glass transition temperature of the binder resin is preferably from 45° C. to 80° C., and more preferably from 55° C. to 70° C. The number average molecular weight (Mn) is preferably from 2,500 to 50,000. The weight average molecular weight (Mw) is preferably from 10,000 to 1,000,000.

The following polyester resins are also preferable as the binder resin.

It is preferable that from 45 mol % to 55 mol % be an alcohol component, and from 45 mol % to 55 mol % be an acid component, based on the total monomer units which constitute a polyester resin.

The acid value of the polyester resin is preferably from 0 mg KOH/g to 90 mg KOH/g, and more preferably from 5 mg KOH/g to 50 mg KOH/g. The hydroxyl value of the polyester resin is preferably from 0 mg KOH/g to 50 mg KOH/g, and more preferably from 5 mg KOH/g to 30 mg KOH/g. This is because when the number of end groups of the molecular chain increases, the charging characteristics of the toner become more dependent on the environment.

The glass transition temperature of the polyester resin is preferably from 50° C. to 75° C., and more preferably from

55° C. to 65° C. The number average molecular weight (Mn) is preferably from 1500 to 50,000, and more preferably from 2000 to 20,000. The weight average molecular weight (Mw) is preferably from 6,000 to 100,000, and more preferably from 10,000 to 90000.

A crystalline polyester resin such as described below may be added to the toner for the purpose of promoting the plasticizing effect of the toner and improving the low-temperature fixability.

10 Examples of crystalline polyesters include polycondensates of monomer compositions including an aliphatic diol having from 2 to 22 carbon atoms and an aliphatic dicarboxylic acid having from 2 to 22 carbon atoms as the main components.

15 The aliphatic diol having from 2 to 22 carbon atoms (more preferably from 6 to 12 carbon atoms) is not particularly limited, but is preferably a chain (more preferably linear) aliphatic diol. Among these, particularly preferred are linear aliphatics such as ethylene glycol, diethylene glycol, 1,4-butanediol and 1,6-hexanediol, and also  $\alpha$ ,  $\omega$ -diols.

20 Among the alcohol components, preferably 50% by mass or more, and more preferably 70% by mass or more is an alcohol selected from aliphatic diols having from 2 to 22 carbon atoms.

25 A polyhydric alcohol monomer other than aliphatic diols can also be used. Examples of the dihydric alcohol monomer include aromatic alcohols such as polyoxyethylenated bisphenol A, polyoxypropyleneated bisphenol A and the like; 1,4-cyclohexanedimethanol and the like.

30 Examples of trivalent or higher polyhydric alcohol monomers include aromatic alcohols such as 1,3,5-trihydroxymethylbenzene and the like; aliphatic alcohols such as pentaerythritol, dipentaerythritol, tripentaerythritol, 1,2,4-butanetriol, 1,2,5-pentanetriol, glycerin, 35 2-methylpropanetriol, 2-methyl-1,2,4-butanetriol, trimethylolethane, trimethylolpropane and the like; and the like.

35 Furthermore, a monovalent alcohol may be used to such an extent that the properties of the crystalline polyester are not impaired.

40 Meanwhile, the aliphatic dicarboxylic acid having from 2 to 22 carbon atoms (more preferably from 6 to 12 carbon atoms) is not particularly limited, but is preferably a chain (more preferably linear) aliphatic dicarboxylic acid. Compounds obtained by hydrolyzing acid anhydrides or lower alkyl esters thereof are also included.

45 Among the carboxylic acid components, preferably 50% by mass or more, and more preferably 70% by mass or more is a carboxylic acid selected from aliphatic dicarboxylic acids having from 2 to 22 carbon atoms.

50 A polyvalent carboxylic acid other than the above-mentioned aliphatic dicarboxylic acids having from 2 to 22 carbon atoms can also be used. Examples of divalent carboxylic acids include aromatic carboxylic acids such as isophthalic acid, terephthalic acid and the like; aliphatic carboxylic acids such as n-dodecylsuccinic acid, n-dodecynylsuccinic acid and the like; and alicyclic carboxylic acids such as cyclohexanedicarboxylic acid and the like. Anhydrides or lower alkyl esters thereof are also included.

55 Examples of trivalent and higher polyvalent carboxylic acids include aromatic carboxylic acids such as 1,2,4-benzenetricarboxylic acid (trimellitic acid), 2,5,7-naphthalene-tricarboxylic acid, 1,2,4-naphthalenetetricarboxylic acid, pyromellitic acid and the like; and aliphatic carboxylic acids such as 1,2,4-butanetricarboxylic acid, 1,2,5-hexanetricarboxylic acid, 1,3-dicarboxyl-2-methyl-2-methylenecarboxypropane and the like. Derivatives and the like thereof such as anhydrides and lower alkyl esters are also included.

Furthermore, a monovalent monohydric carboxylic acid may be also included to such an extent that the characteristics of the crystalline polyester are not impaired.

The crystalline polyester can be produced according to a conventional polyester synthesis method. For example, after the esterification reaction or transesterification reaction of the abovementioned carboxylic acid monomer and alcohol monomer, a desired crystalline polyester is obtained by polycondensation reaction according to a conventional method under reduced pressure or by introducing nitrogen gas.

The amount of the crystalline polyester used is preferably from 0.1 parts by mass to 30 parts by mass, and more preferably from 0.5 parts by mass to 20 parts by mass with respect to 100 parts by mass of the binder resin. Even more preferably, this amount is from 3 parts by mass to 15 parts by mass.

The colorant is preferably nonmagnetic. Examples of the colorant are as follows.

Examples of the black colorant include carbon black and those adjusted to black using a yellow colorant, a magenta colorant and a cyan colorant.

Examples of color pigments for a magenta toner are as follows. Condensed azo compounds, diketopyrrolopyrrole compounds, anthraquinone compounds, quinacridone compounds, basic dye lake compounds, naphthol compounds, benzimidazolone compounds, thioindigo compounds and perylene compounds. Specific examples include C. I. Pigment Red 1, 2, 3, 4, 5, 6, 7, 8, 9, 10, 11, 12, 13, 14, 15, 16, 17, 18, 19, 21, 22, 23, 30, 31, 32, 37, 38, 39, 40, 41, 48:2, 48:3, 48:4, 49, 50, 51, 52, 53, 54, 55, 57:1, 58, 60, 63, 64, 68, 81:1, 83, 87, 88, 89, 90, 112, 114, 122, 123, 144, 146, 150, 163, 166, 169, 177, 184, 185, 202, 206, 207, 209, 220, 221, 238, 254, 269; C. I. Pigment Violet 19, and C. I. Vat Red 1, 2, 10, 13, 15, 23, 29, 35.

Although a pigment may be used alone as a colorant, it is preferable from the viewpoint of the image quality of a full color image to improve the definition by using a dye and a pigment in combination.

Examples of the magenta toner dye are as follows. Oil-soluble dyes such as C. I. Solvent Red 1, 3, 8, 23, 24, 25, 27, 30, 49, 81, 82, 83, 84, 100, 109, 121, C. I. Disperse Read 9, C. I. Solvent Violet 8, 13, 14, 21, 27, and C. I. Disperse Violet 1, and basic dyes such as C. I. Basic Red 1, 2, 9, 12, 13, 14, 15, 17, 18, 22, 23, 24, 27, 29, 32, 34, 35, 36, 37, 38, 39, 40, C. I. Basic Violet 1, 3, 7, 10, 14, 15, 21, 25, 26, 27, 28 and the like.

Examples of the color pigment for a cyan toner are as follows. C. I. Pigment Blue 1, 2, 3, 7, 15:2, 15:3, 15:4, 16, 17, 60, 62, 66; C. I. Vat Blue 6, C. I. Acid Blue 45, and copper phthalocyanine pigments in which from 1 to 5 phthalimidomethyl groups are substituted in the phthalocyanine skeleton.

Examples of color pigments for a yellow toner are as follows. Condensed azo compounds, isoindolinone compounds, anthraquinone compounds, azo metal compounds, methine compounds, allylamine compounds.

Specific examples include C. I. Pigment Yellow 1, 2, 3, 4, 5, 6, 7, 10, 11, 12, 13, 14, 15, 16, 17, 23, 62, 65, 73, 74, 83, 93, 95, 97, 109, 110, 111, 120, 127, 128, 129, 147, 155, 168, 174, 180, 181, 185, 191; and C. I. Vat Yellow 1, 3, 20. Dyes such as C. I. Direct Green 6, C. I. Basic Green 4, C. I. Basic Green 6, Solvent Yellow 162 and the like can also be used.

The amount of the colorant used is preferably from 0.1 parts by mass to 30 parts by mass, more preferably from 0.5 parts by mass to 20 parts by mass, and further preferably

from 3 parts by mass to 15 parts by mass with respect to 100 parts by mass of the binder resin.

A method for producing the toner is not particularly limited, and any known method can be used. For example, a melt-kneading method, a suspension polymerization method, a dissolution suspension method, an emulsion aggregation method and the like can be mentioned.

In the toner, it is preferable to use a binder resin in which a colorant is mixed in advance to make a master batch. Then, 10 the colorant can be well dispersed in the toner by melt-kneading the colorant master batch and other raw materials (binder resin, wax and the like).

A charge control agent can be used, as necessary, to further stabilize the charging performance of the toner. The 15 charge control agent is preferably used in an amount of 0.5 parts by mass to 10 parts by mass per 100 parts by mass of the binder resin. When the amount is 0.5 parts by mass or more, sufficient charging characteristics can be obtained. Meanwhile, when the amount is 10 parts by mass or less, the 20 compatibility with other materials becomes satisfactory, and excessive charging under low humidity can be suppressed.

Examples of the charge control agent are as follows.

For example, an organic metal complex or a chelate compound is effective as a negative charging control agent 25 which controls the toner to be negatively chargeable. Examples thereof include monoazo metal complexes, metal complexes of aromatic hydroxycarboxylic acids, and metal complexes of aromatic dicarboxylic acids. Other examples include aromatic hydroxycarboxylic acids, aromatic mono- and polycarboxylic acids and metal salts thereof, anhydrides thereof, or esters thereof, or phenol derivatives such as bisphenol.

Examples of positive charging control agents that control the toner to be positively chargeable include modified products of nigrosine and fatty acid metal salts, quaternary ammonium salts such as tributylbenzylammonium-1-hydroxy-4-naphthosulfonate, tetrabutylammonium tetrafluoroborate, and the like, onium salts such as phosphonium salts which are analogues thereof, and chelate pigments 40 thereof, triphenylmethane dyes and lake pigments thereof (examples of lake forming agents include phosphotungstic acid, phosphomolybdc acid, phosphotungsten-molybdc acid, tannic acids, lauric acid, gallic acid, ferricyanic acid, ferrocyanide compounds and the like), and examples of metal salts of higher aliphatic acids include diorganotin oxides such as dibutyltin oxide, dioctyltin oxide, dicyclohexyltin oxide and the like, diorganotin borates such as dibutyltin borate, dioctyltin borate, dicyclohexyl tin borate and the like.

If necessary, one or two or more release agents may be contained in the toner particles. The following can be mentioned as a release agent.

Aliphatic hydrocarbon waxes such as low molecular weight polyethylene, low molecular weight polypropylene, 55 microcrystalline wax and paraffin wax can be preferably used. Other examples include oxides of aliphatic hydrocarbon waxes, such as oxidized polyethylene wax, or block copolymers thereof; waxes mainly composed of fatty acid esters such as carnauba wax, sasol wax, montanic acid ester wax and the like; and partially or entirely deoxidized fatty acid esters such as deoxidized carnauba wax and the like.

The amount of the release agent is preferably from 0.1 parts by mass to 20 parts by mass, and more preferably from 0.5 parts by mass to 10 parts by mass with respect to 100 parts by mass of the binder resin.

Moreover, it is preferable that a melting point of a release agent defined by a maximum endothermic peak temperature

at the time of temperature rise measured with a differential scanning calorimeter (DSC) be from 65° C. to 130° C., and more preferably from 80° C. to 125° C. When the melting point is 65° C. or more, the viscosity of the toner is suitable, so that the toner adhesion to the photosensitive member can be suppressed. Meanwhile, when the melting point is 130° C., the low-temperature fixability is improved.

Fine powder that, when externally added to the toner particles, can increase the flowability as compared with that before the addition can be used as a flowability improver of the toner. Examples of suitable fine powders include fluororesin powder such as fine powder of vinylidene fluoride and fine powder of polytetrafluoroethylene; and finely powdered silica such as wet method silica and dry method silica, finely powdered titanium oxide, finely powdered alumina, and the like, subjected to surface treatment and hydrophobized with a silane coupling agent, a titanium coupling agent or silicone oil, and those treated so that the degree of hydrophobization measured by a methanol titration test exhibits a value in the range of from 30 to 80 are particularly preferable.

The inorganic fine particles are preferably used in an amount of from 0.1 parts by mass to 10 parts by mass, and more preferably from 0.2 parts by mass to 8 parts by mass with respect to 100 parts by mass of toner particles.

The two-component developer of the present invention includes a toner having a toner particle including a binder resin, and a magnetic carrier.

When the toner is mixed with the magnetic carrier, the carrier mixing ratio at that time is preferably from 2% by mass to 15% by mass, and more preferably from 4% by mass to 13% by mass, as the toner concentration in the developer, and satisfactory results are usually obtained in these ranges. When the toner concentration is 2% by mass or more, the image density is satisfactory, and when the toner concentration is 15% by mass or less, fogging and scattering inside the machine can be suppressed.

The two-component developer including the magnetic carrier of the present invention can be used in an image forming method which comprises:

a charging step of charging an electrostatic latent image bearing member;

an electrostatic latent image forming step of forming an electrostatic latent image on a surface of the electrostatic latent image bearing member;

a developing step of developing the electrostatic latent image by using a two-component developer in a developing device to form a toner image;

a transfer step of transferring the toner image to a transfer material with or without an intermediate transfer member; and

a fixing step of fixing the transferred toner image to the transfer material.

The image forming method may have a configuration such that the two-component developer is contained in a developing device, and a replenishing developer is supplied to the developing device according to the reduction of the toner concentration of the two-component developer in the developing device. The magnetic carrier of the present invention can be used in the replenishing developer for use in such an image forming method. The image forming method may also have a configuration in which excess magnetic carrier in the developing device is discharged from the developing device as needed.

The replenishing developer preferably includes a magnetic carrier, and a toner having a toner particle including a binder resin and, if necessary, a colorant and a release agent.

The replenishing developer preferably includes from 2 parts by mass to 50 parts by mass of the toner with respect to 1 part by mass of the replenishing magnetic carrier. The replenishing developer may be only the toner, without having the replenishing magnetic carrier.

Next, an image forming apparatus provided with a developing device using a magnetic carrier, a two-component developer and a replenishing developer will be described by way of example, but the present invention is not limited thereto.

#### Image Forming Method

In FIG. 1, an electrostatic latent image bearing member 1 rotates in the direction of the arrow in the figure. The electrostatic latent image bearing member 1 is charged by a charger 2, which is a charging unit, and the surface of the charged electrostatic latent image bearing member 1 is exposed by an exposure unit 3, which is an electrostatic latent image forming unit, to form an electrostatic latent image. The developing device 4 has a developing container 5 for containing a two-component developer, the developer carrying member 6 is rotatably disposed, and magnets 7 are enclosed as a magnetic field generating means inside the developer carrying member 6. At least one of the magnets 7 is installed so as to face the latent image bearing member.

The two-component developer is held on the developer carrying member 6 by the magnetic field of the magnet 7, the amount of the two-component developer is regulated by a regulating member 8, and the two-component developer is transported to a developing unit facing the electrostatic latent image bearing member 1. In the developing unit, a magnetic brush is formed by the magnetic field generated by the magnet 7. Thereafter, the electrostatic latent image is visualized as a toner image by applying a developing bias in which an alternating electric field is superimposed on a DC electric field. The toner image formed on the electrostatic latent image bearing member 1 is electrostatically transferred to a recording medium 12 by a transfer charger 11.

Here, as shown in FIG. 2, the latent image may be temporarily transferred from the electrostatic latent image bearing member 1 to an intermediate transfer member 9 and then electrostatically transferred to a transfer material (recording medium) 12. Thereafter, the recording medium 12 is transported to a fixing device 13, where the toner is fixed on the recording medium 12 by being heated and pressed. Thereafter, the recording medium 12 is discharged as an output image out of the apparatus. After the transfer step, the toner remaining on the electrostatic latent image bearing member 1 is removed by a cleaner 15.

Thereafter, the electrostatic latent image bearing member 1 cleaned by the cleaner 15 is electrically initialized by light irradiation from a pre-exposure 16, and the image forming operation is repeated.

FIG. 2 shows an example of a full color image forming apparatus.

The arrows indicating the arrangement of the image forming units such as K, Y, C, M, and the like and the rotation direction in the figure are not limited to those shown in the figure. Here, K means black, Y means yellow, C means cyan, and M means magenta. In FIG. 2, electrostatic latent image bearing members 1K, 1Y, 1C, 1M rotate in the direction of the arrow in the figure. Each electrostatic latent image bearing member is charged by charging units 2K, 2Y, 2C, 2M as charging means, and on the surface of each electrostatic latent image bearing member that has been charged, exposure is performed with exposure units 3K, 3Y, 3C, 3M as electrostatic latent image forming means to form an electrostatic latent image.

After that, the electrostatic latent image is visualized as a toner image by the two-component developers carried on the developer carrying members 6K, 6Y, 6C, 6M provided in the developing units 4K, 4Y, 4C, 4M, which are developing means. Further, the toner image is transferred to the intermediate transfer member 9 by intermediate transfer chargers 10K, 10Y, 10C, 10M which are transfer means. Further, the image is transferred to the recording medium 12 by the transfer charger 11, which is a transfer means, and the recording medium 12 is outputted as an image after heating and pressurizing with the fixing device 13 which is a fixing means. Then, the intermediate transfer member cleaner 14, which is a cleaning member of the intermediate transfer member 9, recovers the transfer residual toner and the like.

As a developing method, specifically, it is preferable to perform development in a state in which the magnetic brush is in contact with the photosensitive member while applying an alternating voltage to the developer carrying member to form an alternating electric field in the development region. The distance (S-D distance) between the developer carrying member (developing sleeve) 6 and a photosensitive drum of from 100  $\mu\text{m}$  to 1000  $\mu\text{m}$  is satisfactory in preventing carrier adhesion and improving dot reproducibility. Where the distance is 100  $\mu\text{m}$  or more, the supply of the developer is sufficient and the image density is satisfactory. When the distance is 1000  $\mu\text{m}$  or less, magnetic lines from the magnetic pole S1 are unlikely to spread, the density of the magnetic brush becomes satisfactory, and dot reproducibility is improved. In addition, a force restraining the magnetic coat carrier is increased, and the carrier adhesion can be suppressed.

The voltage (Vpp) between the peaks of the alternating electric field is preferably from 300 V to 3000 V, and more preferably from 500 V to 1800 V. The frequency is preferably from 500 Hz to 10,000 Hz, and more preferably from 1000 Hz to 7000 Hz, and can be appropriately selected and used according to the process.

In this case, the waveform of the AC bias for forming the alternating electric field can be exemplified by a triangular wave, a rectangular wave, a sine wave, and a waveform in which the Duty ratio is changed. At the same time, in order to cope with changes in the formation speed of toner images, it is preferable to perform development by applying a developing bias voltage (intermittent alternating superimposed voltage) having a discontinuous AC bias voltage to the developer carrying member. When the applied voltage is 300 V or more, sufficient image density can be easily obtained, and the fog toner in the non-image area can be easily recovered. When the voltage is 3000 V or less, disturbance of the latent image through the magnetic brush is unlikely to occur, and a satisfactory image quality can be obtained.

By using a two-component developer having a toner that has been satisfactorily charged, it is possible to lower the fog removal voltage (Vback) and reduce the primary charge of the photosensitive member, thereby prolonging the life of the photosensitive member. Vback depends on the development system, but is preferably 200 V or less, and more preferably 150 V or less. A potential from 100 V to 400 V is preferably used as a contrast potential so that sufficient image density could be obtained.

Where the frequency is lower than 500 Hz, the electrostatic latent image-bearing member may have the same configuration as the photosensitive member usually used in image forming apparatuses, although the specific configuration is correlated with the process speed. For example, the photosensitive member can be configured by providing a

conductive layer, an undercoat layer, a charge generation layer, a charge transport layer, and, if necessary, a charge injection layer in the order of description on a conductive substrate such as aluminum or SUS.

5 The conductive layer, the undercoat layer, the charge generation layer, and the charge transport layer may be those generally used for a photosensitive member. For example, a charge injection layer or a protective layer may be used as the outermost surface layer of the photosensitive member.

10 Hereafter, methods for measuring the physical properties relating to the present invention are described.

#### Method for Measuring Volume Average Particle Diameter (D50) of Magnetic Carrier and Porous Magnetic Core

15 The particle size distribution is measured by a laser diffraction/scattering type particle size distribution measuring apparatus "MICROTRAC MT3300EX" (manufactured by Nikkiso Co., Ltd.).

20 The measurement of the volume average particle diameter (D50) of the magnetic carrier and porous magnetic core is carried out by attaching a sample feeder for dry measurement "One-shot dry type sample conditioner Turbotrac" (manufactured by Nikkiso Co., Ltd.). The supply conditions of Turbotrac are as follows: a dust collector is used as a vacuum source, the air volume is about 33 L/sec, and the pressure is about 17 kPa. Control is performed automatically on software. As the particle diameter, a 50% particle diameter (D50), which is a cumulative value of volume average, is determined. Control and analysis are performed using provided software (version 10.3.3-202D). The measurement conditions are as follows.

SetZero time: 10 sec

Measurement time: 10 sec

Number of measurements: 1 cycle

Particle refractive index: 1.81%

Particle shape: non-spherical

Upper limit of measurement: 1408  $\mu\text{m}$

Lower limit of measurement: 0.243  $\mu\text{m}$

Measurement environment: 23° C., 50% RH

#### Measurement of Pore Size and Pore Volume of Porous Magnetic Core

The pore size distribution of the porous magnetic core is measured by mercury porosimetry.

45 The measurement principle is as follows.

In this measurement, the pressure applied to mercury is changed, and the amount of mercury penetrated into the pores at that time is measured. The condition under which mercury can penetrate into the pores can be expressed as  $PD = -4\sigma \cos \theta$  from the balance of forces, where P is the pressure, D is the pore diameter, and  $\theta$  and  $\sigma$  are the contact angle and surface tension of mercury, respectively. Assuming that the contact angle and the surface tension are constants, the pressure P and the pore diameter D to which mercury can penetrate at that time are inversely proportional. Therefore, the pressure on the abscissa of a P-V curve obtained by measuring the pressure P and the amount V of the penetrating liquid at that time by changing the pressure is directly converted from this equation into the pore diameter to obtain the pore distribution.

60 Measurement can be performed using a fully automatic multifunction mercury porosimeter PoreMaster series/PoreMaster-GT series manufactured by Yuasa-Ionics Co., an automatic porosimeter AUTOPORE IV 9500 series manufactured by Shimadzu Corporation, or the like as a measuring apparatus.

Specifically, measurement is performed under the following conditions and according to the following procedure by using AUTOPORE IV 9520 manufactured by Shimadzu Corporation.

#### Measurement Conditions

Measurement environment: 20° C.

Measurement cell: sample volume 5 cm<sup>3</sup>, press-fit volume 1.1 cm<sup>3</sup>, application: for powder

Measurement range: from 2.0 psia (13.8 kPa) to 59989.6 psia (413.7 kPa)

Measurement step: 80 steps

(When Taking the Pore Diameter in Logarithm, the Steps are Set so as to be Equally Spaced)

#### Press-Fit Parameter

Exhaust pressure: 50 µm Hg

Exhaust time: 5.0 min

Mercury injection pressure: 2.0 psia (13.8 kPa)

Equilibrium time: 5 secs

#### High-Pressure Parameter

Equilibrium time: 5 secs

#### Mercury Parameter

Advance contact angle: 130.0 degrees

Retracting contact angle: 130.0 degrees

Surface tension: 485.0 mN/m (485.0 dynes/cm)

Mercury density: 13.5335 g/mL

#### Measurement Procedure

(1) About 1.0 g of the porous magnetic core is weighed and put it the sample cell. The weighing value is inputted

(2) The range of from 2.0 psia (13.8 kPa) to 45.8 psia (315.6 kPa) is measured at the low-pressure part.

(3) The range of from 45.9 psia (316.3 kPa) to 59989.6 psia (413.6 kPa) is measured at the high-pressure part.

(4) The pore size distribution is calculated from the mercury injection pressure and the mercury injection amount.

The steps (2), (3), and (4) are automatically performed by software provided with the device.

From the pore diameter distribution measured as described above, the pore diameter at which the differential pore volume in the range of the pore diameter of from 0.1 µm to 3.0 µm is maximized is read and used to set the pore diameter at which the differential pore volume becomes maximal.

Further, the pore volume obtained by integrating the differential pore volume in the range of the pore diameter of from 0.1 µm to 3.0 µm is calculated using the provided software and set as a pore volume.

Separation of Resin Coating Layer from Magnetic Carrier and Fractionation of Resins A and B in Resin Coating Layer

A method in which a magnetic carrier is taken in a cup and a coating resin is eluted using toluene can be used as a method for separating the resin coating layer from the magnetic carrier.

Fractionation is carried out using the following apparatus after drying the eluted resin and then dissolving in tetrahydrofuran (THF).

#### Device Configuration

LC-908 (manufactured by Japan Analytical Industry Co., Ltd.)

JRS-86 (same company; repeat injector)

JAR-2 (same company; auto sampler)

FC-201 (Gilson Co.; Fraction Collector)

#### Column Configuration

JAIGEL-1H to 5H (20φ×600 mm: fractionation column) (manufactured by Japan Analytical Industry Co., Ltd.)

#### Measurement Conditions

Temperature: 40° C.

Solvent: THF

Flow rate: 5 ml/min.

Detector: RI

Based on the molecular weight distribution of the coating resin, the elution time to obtain the peak molecular weight (Mp) of the resin A and the resin B is measured in advance using the resin configuration specified by the following method, and the respective resin components are fractionated theretofore and thereafter. Then, the solvent is removed and drying is performed to obtain the resin A and the resin B.

An atomic group can be specified from an absorption 10 wave number using a Fourier-transform infrared spectroscopic analysis apparatus (Spectrum One: manufactured by PerkinElmer Inc.), and the resin composition of the resin A and the resin B can be specified.

Measurement of Weight Average Molecular Weight (Mw) 15 and Peak Molecular Weight of Resin A, Resin B and Resin Coating Layer, and Content Ratio of Resin A and Resin B in Resin Coating Layer

The weight average molecular weight (Mw) and peak molecular weight of the resin A, resin B, and resin coating 20 layer are measured by the following procedure by using gel permeation chromatography (GPC).

The measurement sample is prepared as follows.

The sample (coating resin separated from the magnetic carrier, or the resin A or the resin B fractionated in the 25 fractionation device) and tetrahydrofuran (THF) are mixed at a concentration of 5 mg/ml and allowed to stand at room temperature for 24 h to dissolve the sample in THF. The solution that was thereafter passed through a sample-treated filter (Mishori Disc H-25-2 manufactured by Tosoh Corporation) is taken as a GPC sample.

Next, using a GPC measurement apparatus (HLC-8120 GPC manufactured by Tosoh Corporation), measurement is performed under the following measurement conditions according to the operation manual of the apparatus.

#### Measurement Conditions

Apparatus: high-speed GPC "HLC-8120 GPC" (manufactured by Tosoh Corporation)

Columns: 7 series of Shodex KF-801, 802, 803, 804, 805, 40 806, 807 (manufactured by Showa Denko K.K.)

Eluent: THF

Flow rate: 1.0 ml/min

Oven temperature: 40.0° C.

Sample injection volume: 0.10 ml

Further, in calculating the weight average molecular 45 weight (Mw) and peak molecular weight (Mp) of the sample, a molecular weight calibration curve generated by standard polystyrene resins (TSK standard polystyrene F-850, F-450, F-288, F-128, F-80, F-40, F-20, F-10, F-4, F-2, F-1, A-5000, A-2500, A-1000, A-500; manufactured by 50 Tosoh Corporation) is used as the calibration curve.

Further, the content ratio is obtained from a peak area ratio in molecular weight distribution measurement. As shown in FIG. 3, when a region 1 and a region 2 are completely separated, the resin content ratio is determined 55 from the area ratio of respective regions. As shown in FIG. 4, in the case where the respective regions overlap, division is made by a line dropped to the horizontal axis vertically from the inflection point of the GPC molecular weight distribution curve, and the content ratio is obtained from the area ratio of the region 1 and the region 2 shown in FIG. 4.

Method for Measuring Weight Average Particle Diameter (D4) and Number Average Particle Diameter (D1)

The weight average particle diameter (D4) and number 60 average particle diameter (D1) of the toner were determined using a precision particle size distribution measuring apparatus (registered trademark, "Coulter Counter Multisizer 3", manufactured by Beckman Coulter, Inc.) based on a pore

electric resistance method and equipped with an aperture tube having a diameter of 100  $\mu\text{m}$  and dedicated software "Beckman Coulter Multisizer 3 Version 3.51" (manufactured by Beckman Coulter, Inc.) which is provided with the apparatus and used to set the measurement conditions and analyze the measurement data. The measurement was performed with 25,000 effective measurement channels, and the measurement data were analyzed and calculated.

A solution prepared by dissolving special grade sodium chloride in ion exchanged water to a concentration of about 1% by mass, for example, "ISOTON II" (trade name) manufactured by Beckman Coulter, Inc., can be used as the electrolytic aqueous solution to be used for measurements.

The dedicated software is set up in the following manner before the measurement and analysis.

The total count number in a control mode is set to 50,000 particles on a "CHANGE STANDARD MEASUREMENT METHOD (SOM) SCREEN" of the dedicated software, the number of measurements is set to 1, and a value obtained using "standard particles 10.0  $\mu\text{m}$ " (manufactured by Beckman Coulter, Inc.) is set as a Kd value. The threshold and the noise level are automatically set by pressing a measurement button of threshold/noise level. Further, the current is set to 1600  $\mu\text{A}$ , the gain is set to 2, the electrolytic solution is set to ISOTON II (trade name), and flush of aperture tube after measurement is checked.

In the "PULSE TO PARTICLE DIAMETER CONVERSION SETTING SCREEN" of the dedicated software, the bin interval is set to a logarithmic particle diameter, the particle diameter bin is set to a 256-particle diameter bin, and a particle diameter range is set from 2  $\mu\text{m}$  to 60  $\mu\text{m}$ .

A specific measurement method is described hereinbelow.

(1) Approximately 200 mL of the electrolytic aqueous solution is placed in a glass 250 mL round-bottom beaker dedicated to Multisizer 3, the beaker is set in a sample stand, and stirring with a stirrer rod is carried out counterclockwise at 24 rpm. Dirt and air bubbles in the aperture tube are removed by the "FLUSH OF APERTURE TUBE" function of the dedicated software.

(2) A total of 30 mL of the electrolytic aqueous solution is placed in a glass 100 mL flat-bottom beaker. Then, about 0.3 mL of a diluted solution obtained by 3-fold mass dilution of "CONTAMINON N" (trade name) (10% by mass aqueous solution of a neutral detergent for washing precision measuring instruments of pH 7 consisting of a nonionic surfactant, an anionic surfactant, and an organic builder, manufactured by Wako Pure Chemical Industries, Ltd.) with ion exchanged water is added as a dispersing agent thereto.

(3) A predetermined amount of ion exchanged water is placed in the water tank of an ultrasonic disperser "Ultrasonic Dispersion System Tetora 150" (manufactured by Nikkaki Bios Co., Ltd.) with an electrical output of 120 W in which two oscillators with an oscillation frequency of 50 kHz are built in with a phase shift of 180 degrees is prepared. About 2 mL of the CONTAMINON N is added to the water tank.

(4) The beaker of (2) hereinabove is set in the beaker fixing hole of the ultrasonic disperser, and the ultrasonic disperser is actuated. Then, the height position of the beaker is adjusted so that the resonance state of the liquid surface of the electrolytic aqueous solution in the beaker is maximized.

(5) About 10 mg of the toner is added little by little to the electrolytic aqueous solution and dispersed therein in a state in which the electrolytic aqueous solution in the beaker of (4) hereinabove is irradiated with ultrasonic waves. Then, the ultrasonic dispersion process is further continued for 60

sec. In the ultrasonic dispersion, the water temperature in the water tank is appropriately adjusted to a temperature from 10° C. to 40° C.

(6) The electrolytic aqueous solution of (5) hereinabove in which the toner is dispersed is dropped using a pipette into the round bottom beaker of (1) hereinabove which has been set in the sample stand, and the measurement concentration is adjusted to be about 5%. Then, measurement is conducted until the number of particles to be measured reaches 50,000.

(7) The measurement data are analyzed with the dedicated software provided with the apparatus, and the weight average particle diameter (D4) and the number average particle diameter (D1) are calculated. The "AVERAGE DIAMETER" on the analysis/volume statistical value (arithmetic mean) screen when the dedicated software is set to graph/volume % is the weight average particle diameter (D4). The "AVERAGE DIAMETER" on the analysis/number statistical value (arithmetic mean) screen when the dedicated software is set to graph/number % is the number average particle diameter (D1).

#### Method for Calculating Fine Powder Amount

The fine powder amount (number %) based on the number of particles in the toner is calculated as follows.

For example, after measuring the number % of particles equal to or less than 4.0  $\mu\text{m}$  in the toner with the Multisizer 3, (1) the dedicated software is set to graph/number % and the chart of the measurement results is displayed as number %. (2) In the particle diameter setting portion on the form/particle diameter/particle diameter statistics screen, "<" is checked, and "4" is inputted to the particle diameter input portion therebelow. Then, (3) the numerical value on the "<4  $\mu\text{m}$ " display part when the analysis/number statistical value (arithmetic mean) screen is displayed is the number % of particles equal to or less than 4.0  $\mu\text{m}$  in the toner.

#### Method for Calculating Coarse Powder Amount

The coarse powder amount (volume %) based on the volume in the toner is calculated as follows.

For example, after measuring the volume % of particles equal to or greater than 10.0  $\mu\text{m}$  in the toner with the Multisizer 3, (1) the dedicated software is set to graph/volume % and the chart of the measurement results is displayed as volume %. (2) In the particle diameter setting portion on the form/particle diameter/particle diameter statistics screen, ">" is checked, and "10" is inputted to the particle diameter input portion therebelow. Then, (3) the numerical value on the ">10  $\mu\text{m}$ " display part when the analysis/volume statistical value (arithmetic mean) screen is displayed is the volume % of particles equal to or greater than 10.0  $\mu\text{m}$  in the toner.

#### Method for Measuring Acid Value of Resin

The acid value is the number of mg of potassium hydroxide required for neutralizing an acid contained in 1 g of the sample. The measurement is performed according to JIS-K0070-1992. The specific measurement procedure is presented hereinbelow.

##### (1) Preparation of Reagents

A total of 1.0 g of phenolphthalein is dissolved in 90 mL of ethyl alcohol (95% by volume), and ion exchanged water is added to make it 100 mL and obtain a phenolphthalein solution.

A total of 7 g of special grade potassium hydroxide is dissolved in 5 mL of water, and ethyl alcohol (95% by volume) is added to make 1 L. The solution is placed in an alkali-resistant container and allowed to stand for 3 days so as to prevent contact with carbon dioxide gas or the like, and then filtering is performed to obtain a potassium hydroxide solution. The obtained potassium hydroxide solution is

stored in an alkali-resistant container. A total of 25 ml of 0.1 mol/l hydrochloric acid is taken into an Erlenmeyer flask, several drops of the phenolphthalein solution are added, titration is performed with the potassium hydroxide solution, and the factor of the potassium hydroxide solution is determined from the amount of the potassium hydroxide solution required for neutralization. The 0.1 mol/L hydrochloric acid is prepared according to JIS K 8001-1998.

(2) Operation

(A) Main Test

A total of 2.0 g of a pulverized resin sample is accurately weighed in a 200 ml Erlenmeyer flask, 100 ml of a mixed solution of toluene/ethanol (2:1) is added, and dissolution is performed over 5 h. Then, several drops of phenolphthalein solution are added as an indicator and titration is performed using a potassium hydroxide solution. The end point of the titration is when the light crimson color of the indicator lasts for about 30 sec.

(B) Blank Test

Titration is performed in the same manner as in the above operation except that no sample is used (that is, only a mixed solution of toluene/ethanol (2:1) is used).

(3) The result obtained is substituted into the following equation to calculate the acid value.

$$A = [(C-B) \times f \times 5.61] / S$$

Here, A is the acid value (mg KOH/g), B is the addition amount (ml) of the potassium hydroxide solution in the blank test, C is the addition amount (ml) of the potassium hydroxide solution in the main test, f is the factor of the potassium hydroxide solution, and S is the mass of the sample (g).

Method for Measuring Hydroxyl Value of Resin

The hydroxyl value is the number of mg of potassium hydroxide required to neutralize acetic acid bonded to a hydroxyl group when acetylating 1 g of the sample. The hydroxyl value of the resin is measured according to JIS K 0070-1992. The specific measurement procedure is presented hereinbelow.

(1) Preparation of Reagents

A total of 25 g of special grade acetic anhydride is placed in a 100 ml volumetric flask, pyridine is added to make the total amount to 100 ml, and thorough shaking is performed to obtain an acetylation reagent. The obtained acetylation reagent is stored in a brown bottle so as not to be exposed to moisture, carbon dioxide and the like.

A total of 1.0 g of phenolphthalein is dissolved in 90 mL of ethyl alcohol (95% by volume), and ion exchanged water is added to make it 100 ml and obtain a phenolphthalein solution.

A total of 35 g of special grade potassium hydroxide is dissolved in 20 ml of water, and ethyl alcohol (95% by volume) is added to make 1 L. The solution is placed in an alkali-resistant container and allowed to stand for 3 days so as to prevent contact with carbon dioxide gas or the like, and then filtering is performed to obtain a potassium hydroxide solution. The obtained potassium hydroxide solution is stored in an alkali-resistant container. A total of 25 ml of 0.5 mol/l hydrochloric acid is taken into an Erlenmeyer flask, several drops of the phenolphthalein solution are added, titration is performed with the potassium hydroxide solution, and the factor of the potassium hydroxide solution is determined from the amount of the potassium hydroxide solution required for neutralization. The 0.5 mol/L hydrochloric acid is prepared according to JIS K 8001-1998.

(2) Operation

(A) Main Test

A total of 1.0 g of a pulverized resin sample is accurately weighed in a 200 ml round bottom flask, and 5.0 ml of the abovementioned acetylation reagent is accurately added thereto using a whole pipet. At this time, when the sample is difficult to dissolve in the acetylation reagent, a small amount of special grade toluene is added for dissolution.

A small funnel is placed on the mouth of the flask and the flask is immersed in a glycerin bath at about 97° C. to about 1 cm from the flask bottom and heated. At this time, in order to prevent the temperature of the neck of the flask from rising due to the heat of the bath, it is preferable to put a cardboard with a round hole on the base of the neck of the flask.

After 1 h, the flask is removed from the glycerin bath and allowed to cool. After cooling, 1 ml of water is added from the funnel followed by shaking to hydrolyze acetic anhydride. The flask is again heated in a glycerin bath for 10 min for complete the hydrolysis. After cooling down, the funnel and the wall of the flask are washed with 5 ml of ethyl alcohol.

A few drops of the phenolphthalein solution are added as an indicator, and titration is performed with the potassium hydroxide solution. The end point of titration is assumed to be when the pale pink color of the indicator lasts for about 30 sec.

(B) Blank Test

Titration is performed in the same manner as in the above operation except that no sample of amorphous polyester is used.

(3) The result obtained is substituted into the following equation to calculate the hydroxyl value.

$$A = [(B-C) \times 28.05 \times f] / S + D$$

Here, A is the hydroxyl value (mg KOH/g), B is the addition amount (ml) of the potassium hydroxide solution in the blank test, C is the addition amount (ml) of the potassium hydroxide solution in the main test, f is the factor of the potassium hydroxide solution, S is the mass of the sample (g), and D is the acid value (mg KOH/g) of the solution.

## EXAMPLES

Hereinafter, the present invention will be more specifically described with reference to examples, but the present invention is not limited to these examples. In the following formulations, parts are by mass unless otherwise specified.

Production Example of Resin A-1

The raw materials listed in Table 1 (total 109.0 parts) were added to a four-neck flask provided with a reflux condenser, a thermometer, a nitrogen suction pipe and an agitation type stirring device, then 100.0 parts of toluene, 100.0 parts of methyl ethyl ketone, and 2.4 parts of azobisisovaleronitrile were added, and the flask was kept at 80° C. for 10 h under nitrogen flow to obtain the solution of a resin (coating resin) A-1 (solid content: 35% by mass).

Resins A-2 to A-11 were obtained in the same manner by using the raw materials listed in Table 1. Physical properties are shown in Table 1.

Production Example of Resin B-1

An autoclave was charged with 50 parts of xylene, purged with nitrogen, and then heated to 185° C. in a sealed state

under stirring. A mixed solution of 100 parts of the raw materials listed in Table 2, 50 parts of di-t-butyl peroxide, and 20 parts of xylene was continuously added dropwise for 3 h, while controlling the temperature inside the autoclave at 185° C., to conduct polymerization. The polymerization was completed by further maintaining the temperature for 1 h, and the solvent was removed to obtain a resin (coating resin) B-1.

Resins B-2 to B-15 and C-1 were obtained in the same manner by using the raw materials listed in Table 2. Physical properties are shown in Table 2.

TABLE 1

| Resin A | Main chain monomer          |                       | Macromonomer          |      |                       |                        |
|---------|-----------------------------|-----------------------|-----------------------|------|-----------------------|------------------------|
|         | Constituting monomers       | Amount added (mass %) | Constituting monomers | Mw   | Amount added (mass %) | Hydroxyl value mgKOH/g |
| A-1     | Cyclohexyl methacrylate     | 75.0                  | Methyl methacrylate   | 5000 | 24.0                  | 57,000 0.0             |
|         | Methyl methacrylate         | 1.0                   |                       |      |                       |                        |
| A-2     | Cyclohexyl methacrylate     | 73.0                  | Methyl methacrylate   | 4000 | 26.8                  | 58,000 0.5             |
|         | 2-Hydroxyethyl methacrylate | 0.2                   |                       |      |                       |                        |
| A-3     | Cyclohexyl methacrylate     | 75.0                  | Methyl methacrylate   | 6000 | 24.7                  | 57,000 0.8             |
|         | 2-Hydroxyethyl methacrylate | 0.3                   |                       |      |                       |                        |
| A-4     | Cyclohexyl methacrylate     | 59.0                  | Methyl methacrylate   | 5000 | 40.0                  | 57,000 0.0             |
|         | Methyl methacrylate         | 1.0                   |                       |      |                       |                        |
| A-5     | Cyclohexyl methacrylate     | 84.0                  | Methyl methacrylate   | 5000 | 15.0                  | 50,000 0.0             |
|         | Methyl methacrylate         | 1.0                   |                       |      |                       |                        |
| A-6     | Cyclohexyl methacrylate     | 47.0                  | Methyl methacrylate   | 5000 | 30.0                  | 65,000 0.0             |
|         | Methyl methacrylate         | 23.0                  |                       |      |                       |                        |
| A-7     | Cyclohexyl methacrylate     | 82.0                  | Methyl methacrylate   | 5000 | 18.0                  | 50,000 0.0             |
|         | —                           |                       |                       |      |                       |                        |
| A-8     | Cyclohexyl methacrylate     | 30.0                  | Methyl methacrylate   | 5000 | 30.0                  | 65,000 0.0             |
|         | Methyl methacrylate         | 40.0                  |                       |      |                       |                        |
| A-9     | Cyclohexyl methacrylate     | 84.0                  | Methyl methacrylate   | 2000 | 16.0                  | 50,000 0.0             |
|         | —                           |                       |                       |      |                       |                        |
| A-10    | Cyclohexyl methacrylate     | 82.0                  | Methyl methacrylate   |      |                       | 50,000 0.0             |
|         | Methyl methacrylate         | 18.0                  |                       |      |                       |                        |
| A-11    | —                           |                       | Methyl methacrylate   | 2000 | 40.0                  | 50,000 0.0             |
|         | Methyl methacrylate         | 60.0                  |                       |      |                       |                        |

In the table, the macromonomers have methacryloyl group at the terminal thereof as a reactive C—C double bond.

TABLE 2

| Resin B | Monomers                    |                       |                            |
|---------|-----------------------------|-----------------------|----------------------------|
|         | Constituting monomers       | Amount added (mass %) | Peak molecular weight (Mp) |
| B-1     | Styrene                     | 95.0                  | 13,000                     |
|         | 2-Hydroxyethyl methacrylate | 2.1                   | 10.0                       |
|         | Methyl methacrylate         | 2.9                   |                            |
| B-2     | Styrene                     | 96.5                  | 13,000                     |
|         | 2-Hydroxyethyl methacrylate | 1.0                   | 5.0                        |
|         | Methyl methacrylate         | 2.5                   |                            |
| B-3     | Styrene                     | 95.0                  | 4,000                      |
|         | 2-Hydroxyethyl methacrylate | 2.5                   | 12.0                       |
|         | Methyl methacrylate         | 2.5                   |                            |
| B-4     | Styrene                     | 95.0                  | 19,000                     |
|         | 2-Hydroxyethyl methacrylate | 2.1                   | 10.0                       |
|         | Methyl methacrylate         | 2.9                   |                            |
| B-5     | Styrene                     | 60.0                  | 13,000                     |
|         | 2-Hydroxyethyl methacrylate | 1.0                   | 5.0                        |
|         | Methyl methacrylate         | 39.0                  |                            |
| B-6     | Styrene                     | 97.9                  | 10,000                     |
|         | 2-Hydroxyethyl methacrylate | 2.1                   | 10.0                       |
|         | —                           | —                     |                            |

TABLE 2-continued

| Resin B | Monomers                    |      | Amount added (mass %) | Peak molecular weight (Mp) | Hydroxyl value (mg KOH/g) |
|---------|-----------------------------|------|-----------------------|----------------------------|---------------------------|
|         | Constituting monomers       |      |                       |                            |                           |
| B-7     | Styrene                     | 96.0 | 10,000                | 2.5                        |                           |
|         | 2-Hydroxyethyl methacrylate | 0.6  |                       |                            |                           |
|         | Methyl methacrylate         | 3.4  |                       |                            |                           |

TABLE 2-continued

| Resin B | Monomers                    |       | Amount added (mass %) | Peak molecular weight (Mp) | Hydroxyl value (mg KOH/g) |
|---------|-----------------------------|-------|-----------------------|----------------------------|---------------------------|
|         | Constituting monomers       |       |                       |                            |                           |
| B-8     | Styrene                     | 95.0  | 5,000                 | 2.0                        |                           |
|         | 2-Hydroxyethyl methacrylate | 0.4   |                       |                            |                           |
|         | Methyl methacrylate         | 4.6   |                       |                            |                           |
| B-9     | Styrene                     | 95.0  | 7,000                 | 13.0                       |                           |
|         | 2-Hydroxyethyl methacrylate | 2.7   |                       |                            |                           |
|         | Methyl methacrylate         | 2.3   |                       |                            |                           |
| B-10    | Styrene                     | 95.0  | 8,000                 | 1.0                        |                           |
|         | 2-Hydroxyethyl methacrylate | 0.2   |                       |                            |                           |
|         | Methyl methacrylate         | 4.8   |                       |                            |                           |
| B-11    | Styrene                     | 95.0  | 10,000                | 15.0                       |                           |
|         | 2-Hydroxyethyl methacrylate | 3.0   |                       |                            |                           |
|         | Methyl methacrylate         | 2.0   |                       |                            |                           |
| B-12    | Styrene                     | 90.0  | 2,800                 | 0.5                        |                           |
|         | 2-Hydroxyethyl methacrylate | 0.1   |                       |                            |                           |
|         | Methyl methacrylate         | 9.9   |                       |                            |                           |
| B-13    | Styrene                     | 90.0  | 21,000                | 20.0                       |                           |
|         | 2-Hydroxyethyl methacrylate | 4.0   |                       |                            |                           |
|         | Methyl methacrylic acid     | 6.0   |                       |                            |                           |
| B-14    | Styrene                     | 100.0 | 5,000                 | 0.0                        |                           |
|         | —                           | 0.0   |                       |                            |                           |
|         | —                           | 0.0   |                       |                            |                           |
| B-15    | —                           | 0.0   | 39,000                | 50.0                       |                           |
|         | 2-Hydroxyethyl methacrylate | 10.0  |                       |                            |                           |
|         | Methyl methacrylate         | 90.0  |                       |                            |                           |

TABLE 2-continued

| Monomers |                       | Amount added (mass %) | Peak molecular weight (Mp) | Hydroxyl value (mg KOH/g) |
|----------|-----------------------|-----------------------|----------------------------|---------------------------|
| Resin B  | Constituting monomers |                       |                            |                           |
| C-1      | —                     | 0.0                   | 28,000                     | 0.0                       |
|          | —                     | 0.0                   |                            |                           |
|          | Methyl methacrylate   | 100.0                 |                            |                           |

## Production Example of Magnetic Carrier Core 1

## Step 1 (Weighing and Mixing Step)

|                                |               |
|--------------------------------|---------------|
| Fe <sub>2</sub> O <sub>3</sub> | 68.3% by mass |
| MnCO <sub>3</sub>              | 28.5% by mass |
| Mg(OH) <sub>2</sub>            | 2.0% by mass  |
| SrCO <sub>3</sub>              | 1.2% by mass  |

The ferrite raw materials were weighed, 20 parts of water was added to 80 parts of the ferrite raw materials, and then wet mixing was performed with a ball mill using zirconia having a diameter ( $\phi$ ) of 10 mm for 3 h to prepare a slurry. The solid fraction concentration of the slurry was 80% by mass.

## Step 2 (Pre-baking Step)

The mixed slurry was dried by a spray dryer (manufactured by Ohkawara Kakohki Co., Ltd.), and then baked for 3.0 h at a temperature of 1050° C. in a nitrogen atmosphere (oxygen concentration 1.0% by volume) in a batch electric furnace to produce a pre-baked ferrite.

## Step 3 (Pulverization Step)

After the pre-baked ferrite was pulverized to about 0.5 mm with a crusher, water was added to prepare a slurry. The solid fraction concentration of the slurry was 70% by mass. Pulverization was then performed for 3 h in a wet ball mill using  $\frac{1}{8}$  inch stainless steel beads to obtain a slurry. The slurry was then pulverized for 4 h in a wet bead mill using zirconia with a diameter of 1 mm to obtain a pre-baked ferrite slurry having a 50% particle diameter (D50) of 1.3  $\mu\text{m}$  on a volume basis.

## Step 4 (Granulation Step)

After adding 1.0 part of ammonium polycarboxylate as a dispersant and 1.5 parts of polyvinyl alcohol as a binder to 100 parts of the pre-baked ferrite slurry, pulverization and drying were performed with a spray dryer (manufactured by Ohkawara Kakohki Co., Ltd.) to obtain spherical particles. The obtained granulated product was adjusted in particle size, and then heated at 700° C. for 2 h by using a rotary electric furnace to remove organic substances such as the dispersant, the binder and the like.

## Step 5 (Baking Step)

Baking was performed in a nitrogen atmosphere (oxygen concentration: 1.0% by volume) by setting the time from room temperature to the baking temperature (1100° C.) to 2 h and holding at a temperature of 1100° C. for 4 h. Thereafter, the temperature was lowered to 60° C. over 8 h, the nitrogen atmosphere was returned to the air atmosphere, and the particles were removed at a temperature of 40° C. or less.

## Step 6 (Sorting Step)

After the aggregated particles were disintegrated, sieving was performed with a sieve of 150  $\mu\text{m}$  to remove coarse particles, air classification was performed to remove fine

particles, and low-magnetic components were further removed by magnetic separation to obtain porous magnetic core particles 1.

## Step 7 (Filling Step)

5 A total of 100 parts of the porous magnetic core particles 1 was placed in a stirring vessel of a mixing stirrer (all-purpose stirrer NDMV type manufactured by Dalton Co., Ltd.), the temperature was maintained at 60° C., and 5 parts of a filling resin including 95% by mass of a methyl silicone oligomer and 5.0% by mass of  $\gamma$ -aminopropyltrimethoxysilane was added dropwise under normal pressure.

After completion of the dropwise addition, stirring was continued while adjusting the time, the temperature was raised to 70° C., and the particles of each porous magnetic core were filled with the resin composition.

15 The resin-filled magnetic core particles obtained after cooling were transferred to a mixer (drum mixer UD-AT type manufactured by Sugiyama Heavy Industries, Ltd.) having a spiral blade in a rotatable mixing container, and the temperature was raised, under stirring, to 140° C. at a temperature rise rate of 2° C./min under a nitrogen atmosphere. Then, heating and stirring were continued at 140° C. for 50 min.

20 After cooling to room temperature, the resin-filled and cured ferrite particles were taken out and nonmagnetic substances were removed using a magnetic separator. Furthermore, coarse particles were removed by a vibrating screen to obtain a magnetic carrier core 1 filled with a resin.

## Production Example of Magnetic Carrier Core 2

25 A total of 4.0 parts of a silane coupling agent (3-(2-aminoethylamino)propyltrimethoxysilane) was added to 100.0 parts of magnetite powder having a number average particle diameter of 0.30  $\mu\text{m}$ , and fine particles were treated by high speed mixing and stirring at 100° C. or higher.

|    |                                                                   |          |
|----|-------------------------------------------------------------------|----------|
| 40 | Phenol                                                            | 10 parts |
|    | Formaldehyde solution (formaldehyde 40%, methanol 10%, water 50%) | 6 parts  |
|    | Treated magnetite                                                 | 84 parts |

45 The above materials, 5 parts of 28% ammonia water and 20 parts of water were placed in a flask, heated and held at 85° C. for 30 min while stirring and mixing to conduct a polymerization reaction for 3 h and cure the generated phenol resin. Thereafter, the cured phenol resin was cooled to 30° C., water was further added, the supernatant was removed, and the precipitate was washed with water and then air dried. Subsequently, drying was performed at a temperature of 60° C. under reduced pressure (5 mm Hg or less) to obtain a spherical magnetic carrier core 2 in a state with a dispersed magnetic substance.

## Production Example of Magnetic Carrier 1

|    |                                  |            |
|----|----------------------------------|------------|
| 60 | Magnetic carrier core 1          | 100 parts  |
|    | Resin A-1 (resin solid fraction) | 0.95 parts |
|    | Resin B-1 (resin solid fraction) | 0.95 parts |

65 The coating resins of the abovementioned numbers of parts, with respect to 100 parts of the magnetic carrier core

1, were diluted with toluene so that each resin component was 5%, and a sufficiently stirred resin solution was prepared as a coating resin 1. Thereafter, the magnetic carrier core 1 was placed in a planetary motion mixer (NAUTA MIXER VN type manufactured by Hosokawa Micron Corporation) maintained at a temperature of 60° C., and the above resin solution was charged. As a method of charging, half of the resin solution was charged, and a solvent removal and coating operation was performed for 30 min. Then, another half of the resin solution was charged, and the solvent removal and coating operation was performed for 40 min.

Thereafter, the magnetic carrier coated with the resin coating layer was transferred to a mixer (drum mixer UD-AT type manufactured by Sugiyama Heavy Industries, Ltd.) having spiral blades in a rotatable mixing container, and heat treated for 2 h at the temperature of 120° C. under nitrogen atmosphere while stirring by rotating at 10 revolutions per 1 min. The resulting magnetic carrier was separated from low magnetic force products by magnetic separation, passed through a sieve with an opening of 150 µm, and then classified with an air classifier to obtain a magnetic carrier 1.

#### Production Examples of Magnetic Carriers 2 to 31

Magnetic carriers 2 to 31 were obtained in the same manner as in Production Example of Magnetic Carrier 1 except that coating resins prepared by changing the combinations of resins and the addition amounts as shown in Table 3 were used and the combinations of magnetic carrier cores shown in Table 5 were used.

TABLE 3

| Coating resin No. | Resin A |                |                    | Resin B |                |                    | Resin C |                    |      |      |
|-------------------|---------|----------------|--------------------|---------|----------------|--------------------|---------|--------------------|------|------|
|                   | No.     | Hydroxyl value | Addition ratio (%) | No.     | Hydroxyl value | Addition ratio (%) | No.     | Addition ratio (%) | PA % | HVC  |
| 1                 | A-1     | 0.0            | 50                 | B-1     | 10.0           | 50                 | —       | —                  | 50   | 5.0  |
| 2                 | A-2     | 0.5            | 50                 | B-1     | 10.0           | 50                 | —       | —                  | 50   | 5.3  |
| 3                 | A-3     | 0.8            | 45                 | B-2     | 5.0            | 55                 | —       | —                  | 46   | 3.1  |
| 4                 | A-1     | 0.0            | 40                 | B-3     | 12.0           | 60                 | —       | —                  | 40   | 7.2  |
| 5                 | A-1     | 0.0            | 50                 | B-4     | 10.0           | 50                 | —       | —                  | 51   | 5.0  |
| 6                 | A-4     | 0.0            | 40                 | B-1     | 10.0           | 60                 | —       | —                  | 40   | 6.0  |
| 7                 | A-5     | 0.0            | 70                 | B-1     | 10.0           | 30                 | —       | —                  | 71   | 3.0  |
| 8                 | A-1     | 0.0            | 45                 | B-1     | 10.0           | 45                 | C-1     | 10                 | 45   | 4.5  |
| 9                 | A-6     | 0.0            | 78                 | B-1     | 10.0           | 22                 | —       | —                  | 79   | 2.2  |
| 10                | A-7     | 0.0            | 45                 | B-3     | 12.0           | 55                 | —       | —                  | 45   | 6.6  |
| 11                | A-8     | 0.0            | 30                 | B-5     | 5.0            | 70                 | —       | —                  | 30   | 3.5  |
| 12                | A-9     | 0.0            | 25                 | B-6     | 10.0           | 75                 | —       | —                  | 25   | 7.5  |
| 13                | A-3     | 0.8            | 37                 | B-3     | 12.0           | 63                 | —       | —                  | 36   | 7.9  |
| 14                | A-1     | 0.0            | 60                 | B-7     | 2.5            | 40                 | —       | —                  | 61   | 1.0  |
| 15                | A-3     | 0.8            | 28                 | B-3     | 12.0           | 72                 | —       | —                  | 29   | 8.9  |
| 16                | A-1     | 0.0            | 50                 | B-8     | 2.0            | 50                 | —       | —                  | 50   | 1.0  |
| 17                | A-1     | 0.0            | 40                 | B-1     | 10.0           | 40                 | C-1     | 20                 | 39   | 4.0  |
| 18                | A-1     | 0.0            | 50                 | B-9     | 13.0           | 50                 | —       | —                  | 51   | 6.5  |
| 19                | A-1     | 0.0            | 50                 | B-10    | 1.0            | 50                 | —       | —                  | 49   | 0.5  |
| 20                | A-1     | 0.0            | 50                 | B-11    | 15.0           | 50                 | —       | —                  | 49   | 7.5  |
| 21                | A-6     | 0.0            | 90                 | B-5     | 5.0            | 10                 | —       | —                  | 91   | 3.0  |
| 22                | A-5     | 0.0            | 20                 | B-6     | 10.0           | 80                 | —       | —                  | 20   | 8.0  |
| 23                | A-1     | 0.0            | 50                 | B-12    | 0.5            | 50                 | —       | —                  | 50   | 0.3  |
| 24                | A-1     | 0.0            | 50                 | B-13    | 20.0           | 50                 | —       | —                  | 50   | 10.0 |
| 25                | A-1     | 0.0            | 90                 | B-12    | 0.5            | 10                 | —       | —                  | 91   | 0.1  |
| 26                | A-1     | 0.0            | 20                 | B-13    | 20.0           | 80                 | —       | —                  | 20   | 16.0 |
| 27                | A-1     | 0.0            | 18                 | B-13    | 20.0           | 82                 | —       | —                  | 18   | 16.4 |
| 28                | A-1     | 0.0            | 99.5               | B-14    | 0.0            | 0.5                | —       | —                  | 99.5 | 0.0  |
| 29                | A-1     | 0.0            | 50                 | B-15    | 50.0           | 50                 | —       | —                  | 51   | 25.0 |
| 30                | A-10    | 0.0            | 50                 | B-13    | 20.0           | 50                 | —       | —                  | 50   | 10.0 |
| 31                | A-11    | 0.0            | 50                 | B-13    | 20.0           | 50                 | —       | —                  | 50   | 10.0 |

In the table, "PA" denotes "Peak area ratio of resin A (%)", and "HVC" denotes "Hydroxyl value of coating resin (mg KOH/g)". The unit of the hydroxyl value in the table is mg KOH/g. The addition ratio is in % by mass.

TABLE 4

| Coating resin No. | Ratio (a) mass % | Ratio (b) mass % | Ratio (c) mass % | Ratio (d) mass % | (a) + (c) |
|-------------------|------------------|------------------|------------------|------------------|-----------|
| 1                 | 37.5             | 12.0             | 47.5             | 1.1              | 85.0      |
| 2                 | 36.5             | 13.4             | 47.5             | 1.1              | 84.0      |
| 3                 | 33.8             | 11.1             | 53.1             | 0.6              | 86.8      |
| 4                 | 30.0             | 9.6              | 57.0             | 1.5              | 87.0      |
| 5                 | 37.5             | 12.0             | 47.5             | 1.1              | 85.0      |
| 6                 | 23.6             | 16.0             | 57.0             | 1.3              | 80.6      |
| 7                 | 58.8             | 10.5             | 28.5             | 0.6              | 87.3      |
| 8                 | 33.8             | 10.8             | 42.8             | 0.9              | 76.5      |
| 9                 | 36.7             | 23.4             | 20.9             | 0.5              | 57.6      |
| 10                | 36.9             | 8.1              | 52.3             | 1.4              | 89.2      |
| 11                | 9.0              | 9.0              | 42.0             | 0.7              | 51.0      |
| 12                | 21.0             | 4.0              | 73.4             | 1.6              | 94.4      |
| 13                | 27.8             | 9.1              | 59.9             | 1.6              | 87.6      |
| 14                | 45.0             | 14.4             | 38.4             | 0.2              | 83.4      |
| 15                | 21.0             | 6.9              | 68.4             | 1.8              | 89.4      |
| 16                | 37.5             | 12.0             | 47.5             | 0.2              | 85.0      |
| 17                | 30.0             | 9.6              | 38.0             | 0.8              | 68.0      |
| 18                | 37.5             | 12.0             | 47.5             | 1.4              | 85.0      |
| 19                | 37.5             | 12.0             | 47.5             | 0.1              | 85.0      |
| 20                | 37.5             | 12.0             | 47.5             | 1.5              | 85.0      |
| 21                | 42.3             | 27.0             | 6.0              | 0.1              | 48.3      |
| 22                | 16.8             | 3.0              | 78.3             | 1.7              | 95.1      |
| 23                | 37.5             | 12.0             | 45.0             | 0.1              | 82.5      |
| 24                | 37.5             | 12.0             | 45.0             | 2.0              | 82.5      |
| 25                | 67.5             | 21.6             | 9.0              | 0.0              | 76.5      |

TABLE 4-continued

| Coating resin No. | Ratio (a) mass % | Ratio (b) mass % | Ratio (c) mass % | Ratio (d) mass % | (a) + (c) |
|-------------------|------------------|------------------|------------------|------------------|-----------|
| 26                | 15.0             | 4.8              | 72.0             | 3.2              | 87.0      |
| 27                | 13.5             | 4.3              | 73.8             | 3.3              | 87.3      |
| 28                | 74.6             | 23.9             | 0.5              | 0.0              | 75.1      |
| 29                | 37.5             | 12.0             | 0.0              | 5.0              | 37.5      |
| 30                | 41.0             | 0.0              | 45.0             | 2.0              | 86.0      |
| 31                | 0.0              | 20.0             | 45.0             | 2.0              | 45.0      |

In the table, Ratio (a) denotes "the proportion (% by mass) of (a) the (meth)acrylic acid ester monomer having an alicyclic hydrocarbon group in the monomers forming the coating resin", Ratio (b) denotes "the proportion (% by mass) of (b) the macromonomer in the monomers forming the coating resin", Ratio (c) denotes "the proportion (% by mass) of (c) the styrene-based monomer in the monomers forming the coating resin", and Ratio (d) denotes "the proportion (% by mass) of (d) the (meth)acrylic acid ester monomer having a hydroxy group and represented by a following formula (1) in the monomers forming the coating resin".

In the table, "(a)+(c)" denotes "the proportion (% by mass) of a sum total of the (meth)acrylic acid ester monomer having an alicyclic hydrocarbon group and the styrene-based monomer".

TABLE 5

|                       | Coating resin        |                           |                              |
|-----------------------|----------------------|---------------------------|------------------------------|
|                       | Magnetic carrier No. | Magnetic carrier core No. | Coated amount, parts by mass |
| Example 1             | 1                    | 1                         | 1 1.9                        |
| Example 2             | 2                    | 1                         | 2 1.9                        |
| Example 3             | 3                    | 1                         | 3 1.9                        |
| Example 4             | 4                    | 1                         | 4 1.9                        |
| Example 5             | 5                    | 1                         | 5 1.9                        |
| Example 6             | 6                    | 1                         | 6 1.9                        |
| Example 7             | 7                    | 1                         | 7 1.9                        |
| Example 8             | 8                    | 1                         | 8 1.9                        |
| Example 9             | 9                    | 1                         | 9 1.9                        |
| Example 10            | 10                   | 1                         | 10 1.9                       |
| Example 11            | 11                   | 1                         | 11 1.9                       |
| Example 12            | 12                   | 1                         | 12 1.9                       |
| Example 13            | 13                   | 1                         | 13 1.9                       |
| Example 14            | 14                   | 2                         | 14 1.9                       |
| Example 15            | 15                   | 2                         | 15 1.9                       |
| Example 16            | 16                   | 2                         | 16 1.9                       |
| Example 17            | 17                   | 2                         | 17 1.9                       |
| Example 18            | 18                   | 2                         | 18 1.9                       |
| Example 19            | 19                   | 1                         | 19 1.9                       |
| Example 20            | 20                   | 1                         | 20 1.9                       |
| Example 21            | 21                   | 1                         | 21 1.9                       |
| Example 22            | 22                   | 1                         | 22 1.9                       |
| Example 23            | 23                   | 1                         | 23 1.9                       |
| Example 24            | 24                   | 2                         | 24 1.9                       |
| Example 25            | 25                   | 2                         | 25 1.9                       |
| Example 26            | 26                   | 2                         | 26 1.9                       |
| Comparative example 1 | 27                   | 2                         | 27 1.9                       |
| Comparative example 2 | 28                   | 2                         | 28 1.9                       |
| Comparative example 3 | 29                   | 2                         | 29 1.9                       |
| Comparative example 4 | 30                   | 2                         | 30 1.9                       |
| Comparative example 5 | 31                   | 2                         | 31 1.9                       |

## Production Example of Toner

Materials shown in Table 6 were thoroughly mixed with a Henschel mixer (FM-75J, manufactured by Nippon Coke

Industry Co., Ltd.), and then kneaded with a twin-screw kneader (trade name: PCM-30, manufactured by Ikegai Iron and Steel Co., Ltd.) set at a temperature of 130° C. at a feed amount of 10 kg/h (kneaded product temperature at discharge was 150° C.). The resulting kneaded product was cooled, coarsely pulverized with a hammer mill, and then finely pulverized with a mechanical pulverizer (trade name: T-250, manufactured by Turbo Kogyo Co., Ltd.) at a feed amount of 15 kg/h. The particles obtained had a weight average particle diameter of 4.9  $\mu\text{m}$ .

The obtained particles were classified using a rotary classifier (trade name: TTSP 100, manufactured by Hosokawa Micron Corporation) to cut fine powder and coarse powder. Cyan toner particles and magenta toner particles were obtained which had a weight average particle diameter of 5.7  $\mu\text{m}$ , a presence ratio of 30.8% by number of particles having a particle diameter of 4.0  $\mu\text{m}$  or less, and a presence ratio of 0.8% by volume of particles having a particle diameter of 10.0  $\mu\text{m}$  or more.

Furthermore, the following materials were introduced into a Henschel mixer (trade name: Model FM-75J, manufactured by Nippon Coke Industry Co., Ltd.), the peripheral speed of the rotating blades was set to 35.0 (m/s), and mixing was performed for 3 min to adhere silica particles and titanium oxide particles to the surface of the cyan toner particles and obtain a cyan toner 1. Similar external addition was also performed with respect to magenta toner particles to obtain a magenta toner 1.

|                                                                                                                                                                                            |           |
|--------------------------------------------------------------------------------------------------------------------------------------------------------------------------------------------|-----------|
| Cyan toner particles 1:                                                                                                                                                                    | 100 parts |
| Silica particles:                                                                                                                                                                          | 3.5 parts |
| (silica particles prepared by the fumed method were surface-treated with 1.5% by mass of hexamethyldisilazane and then adjusted to a desired particle size distribution by classification) |           |
| Titanium oxide particles:                                                                                                                                                                  | 0.7 parts |
| (metatitanic acid having anatase type crystallinity was surface-treated with an octylsilane compound)                                                                                      |           |
| Strontium titanate particles:                                                                                                                                                              | 0.5 parts |
| (surface-treated with an octylsilane compound)                                                                                                                                             |           |

The materials were shaken with a shaker (YS-8D: manufactured by Yayoi Corporation) so that the toner concentration was 8% by using the cyan toner or magenta toner and also magnetic carriers 1 to 29 to prepare 300 g of a two-component developer. The amplitude condition of the shaker was 200 rpm for 2 min.

Meanwhile, 90 parts of the cyan toner or the magenta toner were added to 10 parts of each of magnetic carriers 1 to 29 and mixed for 5 min with a V-type mixer in an environment of normal temperature and humidity 23° C./50% RH to obtain a replenishing developer.

TABLE 6

| Toner particle |                                                                                                                                        |                                                                               |                                                                 |                                                                       |          |
|----------------|----------------------------------------------------------------------------------------------------------------------------------------|-------------------------------------------------------------------------------|-----------------------------------------------------------------|-----------------------------------------------------------------------|----------|
|                | Binder resin<br>(100 parts)                                                                                                            | Colorant                                                                      | Release agent                                                   | Additive                                                              | WT<br>μm |
| Cyan toner     | Polyester resin<br>Tg 58° C.<br>Acid value:<br>15 mgKOH/g<br>Hydroxyl value:<br>15 mgKOH/g<br>Molecular weight:<br>Mn 3500<br>Mw 95000 | C. I. Pigment blue 15:3<br>5.5 parts                                          | Normal paraffin<br>wax<br>6.0 parts<br>Melting point:<br>90° C. | 3,5-Di-t-butyl<br>salicylic acid<br>Aluminum<br>compound<br>0.1 parts | 5.7      |
| Magenta toner  | Polyester resin<br>Tg 58° C.<br>Acid value:<br>15 mgKOH/g<br>Hydroxyl value:<br>15 mgKOH/g<br>Molecular weight:<br>Mn 3500<br>Mw 95000 | C. I. Pigment red 122<br>(6.0 parts)<br>C. I. Pigment red 57:1<br>(1.5 parts) | Normal paraffin<br>wax<br>6.0 parts<br>Melting point:<br>90° C. | 3,5-Di-t-butyl<br>salicylic acid<br>Aluminum<br>compound<br>0.1 parts | 5.7      |

Monomer composition of polyester resin in the table (composition: polyoxypropylene (2.2)-2,2-bis(4-hydroxy-phenyl)propane 40 parts, polyoxyethylene(2.2)-2,2-bis(4-hydroxyphenyl)propane 10 parts, terephthalic acid 40 parts, trimellitic acid anhydride 2 parts, fumaric acid 8 parts).

In the table, "WT" denotes "Weight average particle diameter of toner".

#### Examples 1 to 26 and Comparative Examples 1 to 5

The following evaluation was performed using the obtained two-component developers and replenishing developers.

As an image forming apparatus, a modified color copying machine imagePRESS C850 by Canon Inc. was used.

A two-component developer was placed in each color developing device, replenishing developer containers including the developer for each color replenishment were set, an image was formed, and various evaluations were conducted before and after a durability test.

As a durability test, a chart of FFH output with an image ratio of 5% was used under a printing environment of temperature 23° C./humidity 5 RH % (hereinafter "N/L"), and endurance for 20,000 prints was evaluated. Further, under the printing environment of temperature 30° C./humidity 80 RH % (hereinafter "H/H"), a chart of FFH output with an image ratio of 5% was used, and endurance for 20,000 prints was evaluated.

The FFH, as referred to herein, is a value representing 256 gradations in hexadecimal, 00h being the first gradation (white area) of 256 gradations, and FFH being the 256-th gradation (solid part) of 256 gradations. Conditions

Paper: laser beam printer paper CS-814 (81.4 g/m<sup>2</sup>) (Canon Marketing Japan Co., Ltd.)

Image formation speed: A4 size, full color 85 prints/min

Development conditions: the modification was such that the development contrast could be adjusted to an arbitrary value, and the automatic correction by the main body could not be operated.

Each evaluation item is shown below.

(1) Color Tone Change Under H/H Environment (Evaluation V)

Immediately after conducting the 20,000-print endurance test with an FFH output chart with an image ratio of 5% in the H/H environment, an FFH blue image with a size of 50

mm×50 mm was outputted to the center of A4 size paper (CS-814). At this time, the development contrast of cyan and magenta was adjusted so that the toner laid-on level on the paper was 0.35 mg/cm<sup>2</sup> for both cyan and magenta. The color tone (a\*, b\*) was measured using SpectroScan Transmission (manufactured by GretagMacbeth) to measure a\*; and b\*. After that, 10 prints of the FFH output chart with an image ratio of 40% were outputted in the H/H environment, the FFH blue image with a size of 50 mm×50 mm was outputted to the center of the paper, and the color tone was measured.

The measurement conditions of color tone are as follows.

#### Measurement Conditions

Observation light source: D50

Observation field: 2°

Concentration: DIN NB

White standard: Pap

Filter: None

In general, a\* and b\* are values used in the L\* a\* b\* color system, which is a useful means for quantifying and expressing a color. a\* and b\* both represent the hue. The hue is a scale of color such as red, yellow, green, blue, and purple. Each of a\* and b\* indicates the direction of color, a\* indicates a red-green direction, and b\* indicates a yellow-blue direction. Also, C\* is called saturation which is a measure of vividness of color and is expressed as follows: C\* =  $\{(a^*)^2 + (b^*)^2\}^{1/2}$ .

Among the C\* of the image, a difference between the C\* immediately after the 20,000-print endurance test with the FFH output chart with an image ratio of 5% and the C\* immediately after the 10-print output with the FFH output chart with an image ratio of 40% was taken as  $\Delta C^*$ , and the difference in color tone of the image was evaluated by the  $\Delta C^*$ . The results are shown in Tables 7-1 and 7-2.

A (10 points): 0.00 ≤  $\Delta C^*$  < 0.50

B (9 points): 0.50 ≤  $\Delta C^*$  < 1.00

C (8 points): 1.00 ≤  $\Delta C^*$  < 1.50

D (7 points): 1.50 ≤  $\Delta C^*$  < 2.00

E (6 points): 2.00 ≤  $\Delta C^*$  < 2.50

F (5 points): 2.50 ≤  $\Delta C^*$  < 3.00

G (4 points): 3.00 ≤  $\Delta C^*$  < 3.50

H (3 points): 3.50 ≤  $\Delta C^*$  < 4.00

I (2 points): 4.00 ≤  $\Delta C^*$

## (2) Evaluation of In-plane Uniformity of Halftone in H/H Environment (Evaluation W)

Immediately after conducting the 20,000-print endurance test with the FFH output chart with an image ratio of 5% in the H/H environment, 10 prints of the FFH output chart with an image ratio of 40% were outputted. After that, one 99H output chart (A4 full-surface halftone) with an image ratio of 100% was outputted.

The image density was measured and determined with a spectral densitometer 500 series (manufactured by X-Rite). There was a total of 12 measurement sites:

three points at 5.0 cm, 15.0 cm, and 25.0 cm from the left edge of the image (the earlier printed one is taken as the upper side) at a position at 0.5 cm from the tip of the image (the earlier printed one);

three points at 5.0 cm, 15.0 cm, and 25.0 cm from the left edge of the image at a position at 7.0 cm from the tip of the image;

three points at 5.0 cm, 15.0 cm, and 25.0 cm from the left edge of the image at a position at 14.0 cm from the tip of the image; and

three points at 5.0 cm, 15.0 cm, and 25.0 cm from the left edge of the image at a position at 20.0 cm from the tip of the image, and the difference between the highest image density and the lowest image density was determined. Of the 50 prints, the one with the largest density difference was taken as the evaluation result. The results are shown in Tables 7-1 and 7-2.

A (10 points): less than 0.020

B (9 points): 0.020 or more and less than 0.030

C (8 points): 0.030 or more and less than 0.040

D (7 points): 0.040 or more and less than 0.050

E (6 points): 0.050 or more and less than 0.060

F (5 points): 0.060 or more and less than 0.070

G (4 points): 0.070 or more and less than 0.080

H (3 points): 0.080 or more and less than 0.100

I (2 points): 0.100 or more

## (3) Color Tone Change Under N/L Environment (Evaluation X)

Immediately after conducting the 20,000-print endurance test with the FFH output chart with an image ratio of 5% in the N/L environment, an FFH blue image with a size of 50 mm×50 mm was outputted to the center of A4 size paper (CS-814). At this time, the development contrast of cyan and magenta was adjusted so that the toner laid-on level on the paper was 0.35 mg/cm<sup>2</sup> for both cyan and magenta. The color tone (a\*, b\*) was measured using SpectroScan Transmission (manufactured by GretagMacbeth) to measure a\*; and b\*. After that, 10 prints of the FFH output chart with an image ratio of 40% were outputted in the N/L environment, the FFH blue image with a size of 50 mm×50 mm was outputted to the center of the paper, and the color tone was measured. The evaluation results are shown in Tables 7-1 and 7-2.

The measurement conditions were the same as in the Evaluation V. The difference in color tone of the image was evaluated by the difference ( $\Delta C^*$ ) between the C\* immediately after the 20,000-print endurance test with the FFH output chart with an image ratio of 5% and the C\* immediately after the 10-print output with the FFH output chart with an image ratio of 40%, among the C\* of the image. The results are shown in Tables 7-1 and 7-2.

A (5 points): 0.00≤ $\Delta C^*$ <1.00

B (4 points): 1.00≤ $\Delta C^*$ <2.00

C (3 points): 2.00≤ $\Delta C^*$ <3.00

D (2 points): 3.00≤ $\Delta C^*$ <4.00

E (1 point): 4.00≤ $\Delta C^*$

## (4) Evaluation of In-plane Uniformity of Halftone in N/L Environment (Evaluation Y)

Immediately after conducting the 20,000-print endurance test with the FFH output chart with an image ratio of 5% in the N/L environment, 10 prints of the FFH output chart with an image ratio of 40% were outputted. After that, one 99H output chart (A4 full-surface halftone) with an image ratio of 100% was outputted.

The image density was measured and determined with a spectral densitometer 500 series (manufactured by X-Rite). There were a total of 12 measurement sites:

three points at 5.0 cm, 15.0 cm, and 25.0 cm from the left edge of the image (the earlier printed one is taken as the upper side) at a position at 0.5 cm from the tip of the image (the earlier printed one);

three points at 5.0 cm, 15.0 cm, and 25.0 cm from the left edge of the image at a position at 7.0 cm from the tip of the image;

three points at 5.0 cm, 15.0 cm, and 25.0 cm from the left edge of the image at a position at 14.0 cm from the tip of the image; and

three points at 5.0 cm, 15.0 cm, and 25.0 cm from the left edge of the image at a position at 20.0 cm from the tip of the image, and the difference between the highest image density and the lowest image density was determined. Of the 50 prints, the one with the largest density difference was taken as the evaluation result. The results are shown in Tables 7-1 and 7-2.

A (5 points): less than 0.020

B (4 points): 0.020 or more and less than 0.040

C (3 points): 0.040 or more and less than 0.060

D (2 point): 0.060 or more and less than 0.080

E (1 points): 0.080 or more

## (5) Environmental Difference (Evaluation Z)

Immediately after conducting the 20,000-print endurance test with the FFH output chart with an image ratio of 5% in the H/H environment, an FFH cyan image with a size of 50 mm×50 mm was outputted to the center of A4 size paper (CS-814). At this time, the development contrast obtained at the cyan toner laid-on level on the paper of 0.35 mg/cm<sup>2</sup> was taken as Vh (V).

Meanwhile, immediately after conducting the 20,000-print endurance test with the FFH output chart with an image ratio of 5% in the N/L environment, an FFH cyan image with a size of 50 mm×50 mm was outputted to the center of A4 size paper (CS-814). At this time, the development contrast obtained at the cyan toner laid-on level on the paper of 0.35 mg/cm<sup>2</sup> was taken as V1 (V). Evaluation of environmental difference was performed by the difference (V1-Vh (V)) between the development contrast in the environments. The results are shown in Tables 7-1 and 7-2.

A (10 points): less than 150 V

B (9 points): 150 V or more and less than 170 V

C (8 points): 170 V or more and less than 190 V

D (7 points): 190 V or more and less than 210 V

E (6 points): 210 V or more and less than 230 V

F (5 points): 230 V or more and less than 250 V

G (4 points): 250V or more and less than 270V

H (3 points): 270 V or more and less than 290 V

I (2 points): 290 V or more

## (6) Overall Determination

The evaluation ranks in the evaluation items (1) to (5) were quantified, and the total value was determined according to the following criteria.

In the evaluation items (1), (2) and (5), it was assumed that A=10, B=9, C=8, D=7, E=6, F=5, G=4, H=3, and I=2.

In the evaluation items (3) and (4), it was assumed that A=5, B=4, C=3, D=2, and E=1.

It was determined that the effects of the present invention were obtained when the total value of the overall determination was 20 or more.

The results are shown in Table 8.

TABLE 7-1

| Example | Evaluation V: HH blue color tone (a*, b*) |                 |                          |                     | Evaluation W: HH cyan, |            |         |            |
|---------|-------------------------------------------|-----------------|--------------------------|---------------------|------------------------|------------|---------|------------|
|         | immediately after the                     |                 |                          |                     | HT in-plane uniformity |            |         |            |
|         | After H/H endurance                       | 10-print output | Difference in saturation | Difference in image |                        |            |         |            |
| No.     | a*                                        | b*              | a*                       | b*                  | ΔC                     | Evaluation | density | Evaluation |
| 1       | 11.02                                     | -35.43          | 10.95                    | -35.17              | 0.27                   | A          | 0.013   | A          |
| 2       | 11.05                                     | -35.21          | 10.91                    | -34.94              | 0.30                   | A          | 0.016   | A          |
| 3       | 11.11                                     | -35.30          | 10.92                    | -34.99              | 0.36                   | A          | 0.018   | A          |
| 4       | 11.01                                     | -35.43          | 10.89                    | -35.02              | 0.43                   | A          | 0.022   | B          |
| 5       | 11.02                                     | -35.43          | 10.89                    | -35.06              | 0.39                   | A          | 0.019   | A          |
| 6       | 11.06                                     | -35.43          | 10.87                    | -35.06              | 0.42                   | A          | 0.019   | A          |
| 7       | 11.02                                     | -35.43          | 10.81                    | -35.04              | 0.44                   | A          | 0.031   | C          |
| 8       | 11.05                                     | -35.36          | 10.75                    | -35.01              | 0.46                   | A          | 0.026   | B          |
| 9       | 11.02                                     | -35.43          | 10.55                    | -34.39              | 1.14                   | C          | 0.019   | A          |
| 10      | 11.01                                     | -35.33          | 10.65                    | -34.69              | 0.73                   | B          | 0.033   | C          |
| 11      | 11.02                                     | -35.41          | 10.42                    | -33.86              | 1.66                   | D          | 0.027   | B          |
| 12      | 11.02                                     | -35.44          | 10.86                    | -34.56              | 0.89                   | B          | 0.041   | D          |
| 13      | 11.05                                     | -35.38          | 10.42                    | -34.36              | 1.20                   | C          | 0.038   | C          |
| 14      | 11.02                                     | -35.39          | 10.55                    | -34.76              | 0.79                   | B          | 0.042   | D          |
| 15      | 10.98                                     | -35.37          | 10.65                    | -34.56              | 0.87                   | B          | 0.039   | C          |
| 16      | 11.01                                     | -35.38          | 10.61                    | -34.56              | 0.91                   | B          | 0.043   | D          |
| 17      | 10.77                                     | -35.41          | 10.56                    | -34.46              | 0.97                   | B          | 0.038   | C          |
| 18      | 11.02                                     | -35.37          | 10.63                    | -34.51              | 0.94                   | B          | 0.044   | D          |
| 19      | 10.98                                     | -35.39          | 10.40                    | -34.06              | 1.45                   | C          | 0.051   | E          |
| 20      | 10.97                                     | -35.37          | 10.62                    | -34.48              | 0.96                   | B          | 0.047   | D          |
| 21      | 10.99                                     | -35.36          | 9.85                     | -33.64              | 2.06                   | E          | 0.039   | C          |
| 22      | 10.98                                     | -35.38          | 9.91                     | -33.81              | 1.90                   | D          | 0.045   | D          |
| 23      | 10.99                                     | -35.35          | 9.85                     | -33.78              | 1.94                   | D          | 0.054   | E          |
| 24      | 11.01                                     | -35.36          | 10.01                    | -33.77              | 1.88                   | D          | 0.049   | D          |
| 25      | 10.98                                     | -35.34          | 9.95                     | -33.69              | 1.95                   | D          | 0.051   | E          |
| 26      | 10.97                                     | -35.34          | 9.73                     | -33.52              | 2.20                   | E          | 0.053   | E          |
| C.E. 1  | 10.96                                     | -35.35          | 9.75                     | -32.96              | 2.68                   | F          | 0.061   | F          |
| C.E. 2  | 10.98                                     | -35.34          | 9.81                     | -32.91              | 2.70                   | F          | 0.092   | H          |
| C.E. 3  | 10.96                                     | -35.35          | 9.73                     | -32.75              | 2.88                   | F          | 0.058   | E          |
| C.E. 4  | 10.98                                     | -35.33          | 9.63                     | -32.69              | 2.97                   | F          | 0.074   | G          |
| C.E. 5  | 10.97                                     | -35.30          | 9.41                     | -32.09              | 3.57                   | G          | 0.068   | F          |

In the table, "C.E." denotes "Comparative Example".

TABLE 7-2

| Example | Evaluation X: blue color tone (a*, b*) |                 |                          |                     | Evaluation W: NL cyan, |            |         |               |
|---------|----------------------------------------|-----------------|--------------------------|---------------------|------------------------|------------|---------|---------------|
|         | immediately after the                  |                 |                          |                     | HT in-plane uniformity |            |         |               |
|         | After N/L endurance                    | 10-print output | Difference in saturation | Difference in image |                        |            |         | Environmental |
| No.     | a*                                     | b*              | a*                       | b*                  | ΔC                     | Evaluation | density | Evaluation    |
| 1       | 11.22                                  | -35.43          | 11.55                    | -35.57              | 0.36                   | A          | 0.015   | A             |
| 2       | 11.15                                  | -35.40          | 11.51                    | -35.77              | 0.52                   | A          | 0.013   | A             |
| 3       | 11.13                                  | -35.41          | 11.62                    | -36.37              | 1.08                   | B          | 0.013   | A             |
| 4       | 11.10                                  | -35.45          | 10.54                    | -35.92              | 0.73                   | A          | 0.014   | A             |
| 5       | 11.12                                  | -35.42          | 10.78                    | -34.76              | 0.74                   | A          | 0.015   | A             |
| 6       | 11.18                                  | -35.40          | 10.67                    | -34.06              | 1.43                   | B          | 0.016   | A             |
| 7       | 11.19                                  | -35.41          | 11.05                    | -34.74              | 0.68                   | A          | 0.017   | A             |
| 8       | 11.31                                  | -35.47          | 10.75                    | -34.88              | 0.81                   | A          | 0.017   | A             |
| 9       | 11.10                                  | -35.38          | 11.09                    | -34.09              | 1.29                   | B          | 0.018   | A             |
| 10      | 11.12                                  | -35.36          | 10.55                    | -34.69              | 0.88                   | A          | 0.023   | B             |
| 11      | 11.13                                  | -35.37          | 10.62                    | -34.46              | 1.04                   | B          | 0.019   | A             |
| 12      | 11.12                                  | -35.31          | 10.95                    | -34.56              | 0.77                   | A          | 0.026   | B             |
| 13      | 11.10                                  | -35.35          | 10.92                    | -34.56              | 0.81                   | A          | 0.027   | B             |
| 14      | 11.12                                  | -35.34          | 10.89                    | -34.56              | 0.81                   | A          | 0.033   | B             |
| 15      | 11.13                                  | -35.35          | 10.98                    | -34.21              | 1.15                   | B          | 0.034   | B             |
| 16      | 11.15                                  | -35.33          | 10.88                    | -34.21              | 1.15                   | B          | 0.045   | C             |
| 17      | 11.11                                  | -35.41          | 10.75                    | -34.01              | 1.45                   | B          | 0.029   | B             |
| 18      | 11.10                                  | -35.34          | 10.85                    | -34.19              | 1.18                   | B          | 0.029   | B             |
| 19      | 11.10                                  | -35.31          | 10.78                    | -33.88              | 1.47                   | B          | 0.044   | C             |

(V)  $V_l - V_h$

TABLE 7-2-continued

| Example | Evaluation X: blue color tone (a*, b*) |          |                           |            |            | Evaluation W:<br>NL cyan, |         |            |     |            |
|---------|----------------------------------------|----------|---------------------------|------------|------------|---------------------------|---------|------------|-----|------------|
|         | immediately<br>after the               |          | HT in-plane<br>uniformity |            |            | Environmental             |         |            |     |            |
|         | After N/L                              | 10-print | Difference in             | Difference | difference | V1 – Vh                   |         |            |     |            |
| Example | endurance                              | output   | saturation                | in image   |            |                           |         |            |     |            |
| No.     | a*                                     | b*       | a*                        | b*         | ΔC         | Evaluation                | density | Evaluation | (V) | Evaluation |
| 20      | 11.15                                  | -35.33   | 10.63                     | -33.46     | 1.94       | B                         | 0.033   | B          | 210 | E          |
| 21      | 11.10                                  | -35.32   | 10.52                     | -33.38     | 2.02       | C                         | 0.035   | B          | 185 | C          |
| 22      | 11.10                                  | -35.33   | 10.61                     | -33.46     | 1.93       | B                         | 0.045   | C          | 200 | D          |
| 23      | 11.16                                  | -35.33   | 10.54                     | -33.26     | 2.16       | C                         | 0.046   | C          | 185 | C          |
| 24      | 11.11                                  | -35.30   | 10.28                     | -33.18     | 2.28       | C                         | 0.037   | B          | 235 | F          |
| 25      | 11.12                                  | -35.31   | 10.05                     | -33.06     | 2.49       | C                         | 0.047   | C          | 240 | F          |
| 26      | 11.19                                  | -35.30   | 9.95                      | -33.12     | 2.51       | C                         | 0.039   | B          | 250 | G          |
| C.E. 1  | 11.15                                  | -35.30   | 9.25                      | -32.76     | 3.17       | D                         | 0.039   | B          | 275 | H          |
| C.E. 2  | 11.04                                  | -35.29   | 9.18                      | -33.01     | 2.94       | C                         | 0.061   | D          | 245 | F          |
| C.E. 3  | 11.01                                  | -35.28   | 9.10                      | -32.65     | 3.25       | D                         | 0.063   | D          | 290 | I          |
| C.E. 4  | 11.03                                  | -35.28   | 9.08                      | -33.07     | 2.95       | C                         | 0.067   | D          | 285 | H          |
| C.E. 5  | 11.00                                  | -35.29   | 9.02                      | -35.43     | 3.48       | D                         | 0.068   | D          | 295 | I          |

In the table, "C.E." denotes "Comparative Example".

TABLE 8

| Example | Overall evaluation |    |                 |                 |                 |                 |
|---------|--------------------|----|-----------------|-----------------|-----------------|-----------------|
|         | Evaluation<br>No.  | V  | Evaluation<br>W | Evaluation<br>X | Evaluation<br>Y | Evaluation<br>Z |
| 1       | 10                 | 10 | 5               | 5               | 10              | 40              |
| 2       | 10                 | 10 | 5               | 5               | 10              | 40              |
| 3       | 10                 | 10 | 4               | 5               | 10              | 39              |
| 4       | 10                 | 9  | 5               | 5               | 10              | 39              |
| 5       | 10                 | 10 | 5               | 5               | 9               | 39              |
| 6       | 10                 | 10 | 4               | 5               | 9               | 38              |
| 7       | 10                 | 8  | 5               | 5               | 9               | 37              |
| 8       | 10                 | 9  | 5               | 5               | 8               | 37              |
| 9       | 8                  | 10 | 4               | 5               | 9               | 36              |
| 10      | 9                  | 8  | 5               | 4               | 9               | 35              |
| 11      | 7                  | 9  | 4               | 5               | 9               | 34              |
| 12      | 9                  | 7  | 5               | 4               | 9               | 34              |
| 13      | 8                  | 8  | 5               | 4               | 9               | 34              |
| 14      | 9                  | 7  | 5               | 4               | 9               | 34              |
| 15      | 9                  | 8  | 4               | 4               | 7               | 32              |
| 16      | 9                  | 7  | 4               | 3               | 9               | 32              |
| 17      | 9                  | 8  | 4               | 4               | 7               | 32              |
| 18      | 9                  | 7  | 4               | 4               | 7               | 31              |
| 19      | 8                  | 6  | 4               | 3               | 9               | 30              |
| 20      | 9                  | 7  | 4               | 4               | 6               | 30              |
| 21      | 6                  | 8  | 3               | 4               | 8               | 29              |
| 22      | 7                  | 7  | 4               | 3               | 7               | 28              |
| 23      | 7                  | 6  | 3               | 3               | 8               | 27              |
| 24      | 7                  | 7  | 3               | 4               | 5               | 26              |
| 25      | 7                  | 6  | 3               | 3               | 5               | 24              |
| 26      | 6                  | 6  | 3               | 4               | 4               | 23              |
| C.E. 1  | 5                  | 5  | 2               | 4               | 3               | 19              |
| C.E. 2  | 5                  | 3  | 3               | 2               | 5               | 18              |
| C.E. 3  | 5                  | 6  | 2               | 2               | 2               | 17              |
| C.E. 4  | 5                  | 4  | 3               | 2               | 3               | 17              |
| C.E. 5  | 4                  | 5  | 2               | 2               | 2               | 15              |

In the table, "C.E." denotes "Comparative Example".

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2018-149544, filed Aug. 8, 2018, which is hereby incorporated by reference herein in its entirety.

What is claimed is:

1. A magnetic carrier comprising a magnetic carrier particle,  
wherein  
the magnetic carrier particle contains  
a magnetic carrier core and  
a resin coating layer formed on a surface of the magnetic carrier core,

the resin coating layer includes a resin component including a resin A and a resin B, the resin A is a copolymer of monomers including (a) a (meth)acrylic acid ester monomer having an alicyclic hydrocarbon group, and (b) a macromonomer containing a polymer portion and a reactive portion bound to the polymer portion, wherein the polymer portion has a polymer of at least one monomer selected from the group consisting of methyl acrylate, methyl methacrylate, butyl acrylate, butyl methacrylate, 2-ethylhexyl acrylate and 2-ethylhexyl methacrylate, and the reactive portion has a reactive C—C double bond, the resin B is a copolymer of monomers including (c) a styrene-based monomer, and (d) a (meth)acrylic acid ester monomer having a hydroxy group and represented by a following formula (1), and based on the resin components of the resin coating layer, the amount of the resin A is from 20% by mass to 99% by mass, and the amount of the resin B is from 1% by mass to 80% by mass,



wherein, R represents H or CH<sub>3</sub>, and n represents an integer of from 1 to 8.

2. The magnetic carrier according to claim 1, wherein the sum total of the amount of the resin A and the amount of the resin B is from 80% by mass to 100% by mass based on the resin component.

3. The magnetic carrier according to claim 1, wherein a hydroxyl value of the resin component included in the resin coating layer is from 0.5 mg KOH/g to 10.0 mg KOH/g.

4. The magnetic carrier according to claim 1, wherein based on the mass of the monomers forming the resin component included in the resin coating layer, the proportion of the (meth)acrylic acid ester monomer having an alicyclic hydrocarbon group is from 5.0% by mass to 80.0% by mass, the proportion of the styrene-based monomer is from 0.8% by mass to 70.0 by mass, and the proportion of a sum total of the (meth)acrylic acid ester monomer having an alicyclic hydrocarbon group and the styrene-based monomer is from 50.0% by mass to 95.0 by mass.

5. The magnetic carrier according to claim 1, wherein based on the mass of the monomers forming the resin component included in the resin coating layer, the proportion of the (meth)acrylic acid ester monomer having a hydroxy group and represented by the formula (1) is from 0.1% by mass to 3.0% by mass.

6. The magnetic carrier according to claim 1, wherein the hydroxyl value of the resin B is from 0.2 mg KOH/g to 30.0 mg KOH/g.

7. The magnetic carrier according to claim 1, wherein the hydroxyl value of the resin A is from 0 mg KOH/g to 1.0 mg KOH/g.

8. The magnetic carrier according to claim 1, wherein peak molecular weight in a molecular weight distribution of the resin B determined by gel permeation chromatography (GPC) is from 3000 to 20,000.

9. The magnetic carrier according to claim 1, wherein the proportion of the macromonomer is from 15.0% by mass to 40.0% by mass based on the mass of the monomers for forming the resin A.

5 10. An image forming method comprising: a charging step of charging an electrostatic latent image bearing member; an electrostatic latent image forming step of forming an electrostatic latent image on a surface of the electrostatic latent image bearing member; a developing step of developing the electrostatic latent image by using a two-component developer to form a toner image; a transfer step of transferring the toner image to a transfer material with or without an intermediate transfer member; and a fixing step of fixing the transferred toner image to the transfer material,

wherein the two-component developer comprises a toner having a toner particle including a binder resin, and a magnetic carrier, wherein the magnetic carrier is the magnetic carrier according to claim 1.

11. A replenishing developer for use in an image forming method which comprises: a charging step of charging an electrostatic latent image bearing member; an electrostatic latent image forming step of forming an electrostatic latent image on a surface of the electrostatic latent image bearing member; a developing step of developing the electrostatic latent image by using a two-component developer in a developing device to form a toner image; a transfer step of transferring the toner image to a transfer material with or without an intermediate transfer member; and a fixing step of fixing the transferred toner image to the transfer material, and in which a replenishing developer is replenished to the developing device in accordance with a reduction in toner concentration in the two-component developer in the developing device, wherein the replenishing developer includes a magnetic carrier and a toner having a toner particle including a binder resin, the replenishing developer includes from 2 parts by mass to 50 parts by mass of the toner with respect to 1 part by mass of the magnetic carrier, and the magnetic carrier is the magnetic carrier according to claim 1.

12. An image forming method which comprises: a charging step of charging an electrostatic latent image bearing member; an electrostatic latent image forming step of forming an electrostatic latent image on a surface of the electrostatic latent image bearing member; a developing step of developing the electrostatic latent image by using a two-component developer in a developing device to form a toner image; a transfer step of transferring the toner image to a transfer material with or without an intermediate transfer member; and a fixing step of fixing the transferred toner image to the transfer material, and in which a replenishing developer is replenished to the developing device in accordance with a reduction in

45

toner concentration in the two-component developer in the developing device, wherein the replenishing developer includes a magnetic carrier and a toner having a toner particle including a binder resin, the replenishing developer includes from 2 parts by mass to 50 parts by mass of the toner with respect to 1 part by mass of the magnetic carrier, and the magnetic carrier is the magnetic carrier according to claim 1.

13. A two-component developer comprising  
a toner having a toner particle including a binder resin,  
and  
a magnetic carrier,  
wherein  
the magnetic carrier comprises a magnetic carrier particle,  
the magnetic carrier particle has  
a magnetic carrier core and  
a resin coating layer formed on a surface of the mag-  
netic carrier core,  
wherein  
the resin coating layer includes a resin component includ-  
ing a resin A and a resin B,  
the resin A is a copolymer of monomers including  
(a) a (meth)acrylic acid ester monomer having an alicyclic  
hydrocarbon group, and

46

(b) a macromonomer containing a polymer portion and a reactive portion bound to the polymer portion, wherein the polymer portion has a polymer of at least one monomer selected from the group consisting of methyl acrylate, methyl methacrylate, butyl acrylate, butyl methacrylate, 2-ethylhexyl acrylate and 2-ethylhexyl methacrylate, and

the reactive portion has a reactive C—C double bond, the resin B is a copolymer of monomers including

(c) a styrene-based monomer, and

(d) a (meth)acrylic acid ester monomer having a hydroxy group and represented by a following formula (1), and based on the resin components of the resin coating layer, the amount of the resin A is from 20% by mass to 99% by mass, and the amount of the resin B is from 1% by mass to 80% by mass,



(1)

wherein, R represents H or  $\text{CH}_3$ , and n represents an integer of from 1 to 8.

\* \* \* \*